



US011926804B1

(12) **United States Patent**  
**Donham et al.**

(10) **Patent No.:** US 11,926,804 B1  
(45) **Date of Patent:** Mar. 12, 2024

(54) **DISPERSANT AND DETERGENT SYSTEMS  
FOR IMPROVED MOTOR OIL  
PERFORMANCE**

2203/003; C10M 2217/028; C10M  
2219/046; C10M 2223/045; C10M  
2229/00; C10N 2030/68; C10N 2030/52;  
C10N 2030/041; C10N 2030/06; C10N  
2030/10; C10N 2040/25

See application file for complete search history.

(71) Applicant: **Afton Chemical Corporation**,  
Richmond, VA (US)

(72) Inventors: **Leah Donham**, Henrico, VA (US);  
**Kongsheng Yang**, Glen Allen, VA (US);  
**Kenneth Garelick**, Mechanicsville, VA  
(US); **Kristi Engelman**, Richmond, VA  
(US)

(73) Assignee: **Afton Chemical Corporation**,  
Richmond, VA (US)

(\*) Notice: Subject to any disclaimer, the term of this  
patent is extended or adjusted under 35  
U.S.C. 154(b) by 0 days.

(21) Appl. No.: **18/162,331**

(22) Filed: **Jan. 31, 2023**

(51) **Int. Cl.**

**C10M 169/04** (2006.01)  
**C10M 135/10** (2006.01)

(Continued)

(52) **U.S. Cl.**

CPC ..... **C10M 169/041** (2013.01); **C10M 135/10**  
(2013.01); **C10M 137/10** (2013.01); **C10M  
141/10** (2013.01); **C10M 149/10** (2013.01);  
**C10M 155/00** (2013.01); **C10M 157/10**  
(2013.01); **C10M 2203/003** (2013.01); **C10M  
2217/028** (2013.01); **C10M 2219/046**  
(2013.01); **C10M 2223/045** (2013.01); **C10M  
2229/00** (2013.01); **C10N 2030/041** (2020.05);  
(Continued)

(58) **Field of Classification Search**

CPC ..... C10M 169/041; C10M 135/10; C10M  
137/10; C10M 141/10; C10M 149/10;  
C10M 155/00; C10M 157/10; C10M

(56)

**References Cited**

U.S. PATENT DOCUMENTS

1,857,214 A 5/1932 Rowe  
2,995,569 A 8/1961 Hamilton et al.  
(Continued)

FOREIGN PATENT DOCUMENTS

EP 612839 A1 8/1994  
EP 0894845 A1 2/1999  
(Continued)

OTHER PUBLICATIONS

Huanmou et al., "Lubricity of Carboxyl Acid Derivatives of O,O-dialkyl-phosphorodithioate," Journal of Hunan University, vol. 23, No. 3, (1996), pp. 65-70.

Primary Examiner — Vishal V Vasisth

(74) Attorney, Agent, or Firm — Honigman LLP

(57)

**ABSTRACT**

The present disclosure relates to passenger car motor oil lubricating oil compositions having select dispersant and detergent systems to improve at least one of deposits, sludge, oxidization, and wear when using a blend of API Group II base oils with one or more API Group III and/or API Group IV base oils. The dispersant systems herein includes select amounts of boron, nitrogen, and total base number contributions that surprisingly achieve performance even when including higher amounts of the API Group II base oils in the lubricants.

**18 Claims, 2 Drawing Sheets**



US 11,926,804 B1

Page 2

\* cited by examiner



FIG. 1



FIG. 2



FIG. 3

**DISPERSANT AND DETERGENT SYSTEMS  
FOR IMPROVED MOTOR OIL  
PERFORMANCE**

**TECHNICAL FIELD**

The present disclosure relates to additive packages for lubricating compositions and, in particular, dispersant and detergent systems for improved performance in passenger car motor oil lubricating compositions.

**BACKGROUND**

Automotive manufacturers continue to the push for improved efficiency, fluid longevity, and fuel economy, and as such, demands on engines, lubricants, and their components continue to increase. These requirements also mean engine oil performance must evolve to meet the higher demands of such modern engines and their corresponding performance criteria tied to their unique use and applications. With such exacting demands for engine oils, lubricant manufacturers often tailor lubricants and their additives to meet certain performance requirements for industry and/or manufacturer applications. Typically, industry standards and/or automotive manufacturers require certain performance standards such that a lubricant designed for one use or application may not satisfy all the performance specifications for a different use or application.

The American Petroleum Institute (API) classifies base stocks for lubricants into five groups with API Groups I, II, and III defining mineral oil base stocks categorized by saturates, sulfur, and viscosity index. API Group IV relates to polyalphaolefin base stocks, and API Group V includes all other base stocks. In the context of mineral oil base stocks, it is generally appreciated that the performance a mineral oil base stock provides to a lubricant increases from Group I to Group III where the API Group III base stocks being the more-preferred in terms of quality with the Group I and the Group II base stocks tending to provide one or more performance debits under modern industry performance testing. As such, the trend in the lubricant industry has been to use higher amounts of the API Group III base stock when formulating lubricants to meet the strict demands of today's industry and automotive standards.

**SUMMARY**

The present disclosure relates to a passenger car motor oil lubricating composition suitable for improving at least one of deposits, sludge, oxidization, and wear. In one approach or embodiment, the passenger car motor oil lubricating composition includes a blend of base oils of lubricating viscosity including one or more API Group II base oils and one or more API Group III base oils and/or one or more API Group IV base oils; oil soluble nitrogen-containing dispersant additives comprising (i) at least one boronated oil soluble nitrogen-containing dispersant additive and (ii) at least one non-boronated oil soluble nitrogen-containing dispersant additive wherein the oil soluble nitrogen-containing dispersant additives provide an amount of dispersant boron (B), an amount of dispersant nitrogen (N), and a dispersant total base number (TBN) to the passenger car motor oil lubricating composition; metal-containing detergent additives including (i) at least one calcium-containing detergent additive and (ii) at least one magnesium-containing detergent additive; and wherein the passenger car motor oil lubricating composition has a ratio of the dispersant boron,

the dispersant nitrogen, and the dispersant TBN provided by the dispersant formula B/(N\*TBN) of less than 0.25 and, more preferably, wherein the dispersant formula B/(N\*TBN) is less than 0.2.

- 5 In other embodiments or approaches, the passenger car motor oil lubricating composition of the previous paragraph can be combined with optional features or embodiments in any combination. These optional features or embodiments include one or more of the following: wherein the blend of  
10 base oils includes at least about 25 weight percent of the one or more API Group II base oils; and/or wherein the blend of base oils includes at least about 50 weight percent of the one or more API Group II base oils; and/or wherein the blend of base oils is about 25 to about 80 weight percent of the one or more API Group II base oils and about 20 to about 75 weight percent of the one or more API Group III base oils; and/or wherein the oil soluble nitrogen-containing dispersant additives provide no more than about 250 ppm of the dispersant boron to the passenger car motor oil lubricating  
15 composition; and/or wherein the oil soluble nitrogen-containing dispersant additives provide no more than about 200 ppm of the dispersant boron to the passenger car motor oil lubricating composition; and/or wherein the dispersant TBN of the oil soluble nitrogen-containing dispersant additives is about 1.0 to about 1.28 mg KOH/gram as measured pursuant to ASTM D2896; and/or wherein the at least one boronated oil soluble nitrogen-containing dispersant additive provides up to 230 ppm dispersant boron and wherein the nitrogen-containing dispersant additives provide up to 700 ppm dispersant nitrogen; and/or wherein the at least one boronated oil soluble nitrogen-containing dispersant additive provides up to 200 ppm dispersant boron and wherein the nitrogen-containing dispersant additives provide up to 650 ppm dispersant nitrogen; and/or wherein the metal-containing  
20 detergents provide an amount of calcium soap and an amount of magnesium soap to the passenger car motor oil lubricating composition and wherein the passenger car motor oil lubricating composition has more calcium soap than magnesium soap; and/or wherein the metal-containing detergents have a weight ratio of the calcium soap to the magnesium soap of up to about 1.6:1; and/or wherein the metal-containing detergents have a weight ratio of the calcium soap to the magnesium soap of up to about 1.4:1; and/or wherein the metal-containing detergents are substantially free of detergent additives providing phenate soap; and/or wherein the passenger car motor oil lubricating composition has an average engine sludge (AES) of at least about 7.6 merits as measured pursuant to ASTM D8256; and/or wherein the passenger car motor oil lubricating composition has an average weighted piston deposits of at least 5.3 merits as measured pursuant to GMW-17043; and/or further including a viscosity index improver having a shear stability index (SSI) of less than 50 as measured pursuant to ASTM D6278; and/or wherein the viscosity index improver is a non-dispersant viscosity index improver selected from polyolefins, olefin copolymers, ethylene/propylene copolymers, polyisobutenes, hydrogenated styrene-isoprene polymers, styrene/maleic ester copolymers, hydrogenated styrene/butadiene copolymers, hydrogenated isoprene polymers, alpha-olefin maleic anhydride copolymers, polymethacrylates, polyacrylates, polyalkyl styrenes, hydrogenated alkenyl aryl conjugated diene copolymers, and mixtures thereof; and/or wherein the lubricating composition has a sulfated ash (SASH) content of no more than about 0.9 weight percent as measured pursuant to ASTM D874; and/or wherein the lubricating composition has a sulfated ash (SASH) content of no more than about 0.8

weight percent as measured pursuant to ASTM D874; and/or further including one or more metal dihydrocarbyl dithiophosphate compounds, wherein the hydrocarbyl groups thereof are derived from a mixture of secondary alcohols and primary alcohols and with a ratio of the primary alcohols to the secondary alcohols of about 0.3:1 to about 0.6:1; and/or wherein an average number of carbon atoms in the hydrocarbyl groups per primary alcohol is no more than about 0.6:1.

In another approach or embodiment, the present disclosure provides for methods of lubricating an internal combustion engine with a passenger car motor oil wherein the passenger car motor oil is any embodiment or approach as described in this Summary.

In another approach or embodiment, the present disclosure also provides for the use of a passenger car motor oil lubricating composition including a blend of base oils of lubricating viscosity including one or more API Group II base oils and one or more API Group III base oils and/or one or more API Group IV base oils; oil soluble nitrogen-containing dispersant additives comprising (i) at least one boronated oil soluble nitrogen-containing dispersant additive and (ii) at least one non-boronated oil soluble nitrogen-containing dispersant additive wherein the oil soluble nitrogen-containing dispersant additives provide an amount of dispersant boron (B), an amount of dispersant nitrogen (N), and a dispersant total base number (TBN) to the passenger car motor oil lubricating composition; metal-containing detergent additives including (i) at least one calcium-containing detergent additive and (ii) at least one magnesium-containing detergent additive; and wherein the passenger car motor oil lubricating composition has a ratio of the dispersant boron, the dispersant nitrogen, and the dispersant TBN provided by the dispersant formula  $B/(N^*TBN)$  of less than 0.25 and, more preferably, wherein the dispersant formula  $B/(N^*TBN)$  is less than 0.2, and for achieving an average engine sludge (AES) of at least about 7.6 merits as measured pursuant to ASTM D8256 and/or for achieving an average weighted piston deposits of at least 5.3 merits as measured pursuant to GMW-17043

#### BRIEF DESCRIPTION OF DRAWING FIGURES

FIG. 1 is a graph of average Weighted Piston Deposits (WPD) pursuant to GMW-17043 based on the weight percent of the API Group II and Group III base oil amounts in the base oil blend;

FIG. 2 is a graph of Average Engine Sludge (AES) pursuant to ASTM D8256 in a 5W-30 passenger car motor oil based on the weight percent of the API Group II and Group III base oil amounts in the base oil blend; and

FIG. 3 is a graph of Average Engine Sludge (AES) pursuant to ASTM D8256 in a 0W-20 passenger car motor oil based on the weight percent of the API Group II and Group III base oil amounts in the base oil blend.

#### DETAILED DESCRIPTION

The present disclosure relates to passenger car motor oils, and in particular, passenger car motor oils including increased amounts of API Group II base stocks that still achieve strong performance in terms of deposits, sludge, oxidation and/or wear pursuant to modern industry performance testing. Surprisingly, it was discovered that performance debits when using the less-desired API Group II base stocks could be overcome when select relationships of boron, nitrogen, and total base number (TBN) provided by

oil soluble nitrogen-containing dispersant additives in the lubricant was carefully controlled when combined with the less-desired API Group II base oil in the base oil blend.

In particular, the passenger car motor oil lubricating compositions herein include a blend of base oils of lubricating viscosity including one or more API Group II base oil combined with one or more API Group III base oil and/or one or more API Group IV base oils. Preferably, the blend of base oils is at least about 25 weight percent of the one or 10 more API Group II base oils, at least about 50 weight percent of the one or more API Group II base oil, and, more preferably, may include about 25 to about 80 weight percent of the API Group II base oils and about 20 to about 75 weight percent of the API Group III base oils. While API 15 Group II base oils have been available for many years, recent requirements of modern engine performance tests, such as the oxidization and deposit test of GMW-17043, the Sequence VH engine test of ASTM D8256, and others, often demanded by industry and/or automotive manufacturers 20 means that higher levels of API Group II base oil were no longer capable of meeting the heightened performance demands of these new standards.

However, it was surprisingly discovered that even with higher levels of the less-desired API Group II base oil, any 25 performance debit from the base oil could be overcome if the passenger car motor oil lubricating composition has a ratio of the dispersant boron (B), the dispersant nitrogen (N), and the dispersant total base number (TBN) provided by the dispersant formula  $B/(N^*TBN)$  of about 0.25 or less, and 30 preferably about 0.2 or less. In other approaches, the dispersants herein also provide no more than about 250 ppm of boron to the passenger car motor oil lubricating composition, no more than about 230 ppm of boron, or no more than about 200 ppm of boron. The passenger car motor oil 35 lubricating compositions herein, for example and even including a blend of API Group II base oils with API Group III and/or Group IV base oils, still exhibits an average engine sludge (AES) rating of at least about 7.6 merits pursuant to ASTM D8256 and an average weighted piston deposit (WPD) rating of at least about 5.3 merits as measured 40 pursuant to GMW-17043.

#### Dispersant System

The dispersant system of the passenger car motor oil lubricating compositions herein includes one or more oil 45 soluble nitrogen-containing compounds. Preferably, the dispersant system includes (i) at least one or more boronated oil soluble nitrogen-containing dispersant additives and (ii) at least one non-boronated oil soluble nitrogen-containing dispersant additives where the additives of the detergent system combine to provide a total amount of dispersant boron (B), a total amount of dispersant nitrogen (N), and a dispersant total base number (TBN as measured via ASTM D2896). As noted above to achieve performance when combined with API Group II base oils, the lubricants herein have a ratio of 50 the dispersant boron (B), the dispersant nitrogen (N), and the dispersant TBN provided by the formula  $B/(N^*TBN)$  of less than about 0.25, preferably less than about 0.2, or alternatively, about 0.1 to about 0.25 or about 0.12 to about 0.2.

In approaches, the dispersant system provides up to about 60 250 ppm of boron, up to about 230 ppm of boron, or up to about 200 ppm of boron. In other approaches, the dispersant system may provide about 100 ppm to about 250 ppm of boron, about 100 ppm to about 230 ppm of boron, or about 100 ppm to about 200 ppm of boron.

In other approaches, the dispersant system herein may 65 also provide up to about 700 ppm of nitrogen, up to about 680 ppm of nitrogen, or up to about 650 ppm of nitrogen. In

other approaches, the dispersant system herein may provide about 500 ppm to about 700 ppm of nitrogen, about 500 ppm to about 680 ppm of nitrogen, or about 500 ppm to about 650 ppm of nitrogen.

In yet other approaches, the dispersant system herein has a total base number (TBN) as measured pursuant to ASTM D2896 of about 1.0 to about 1.28 mg KOH/gram, and in other approaches, about 1.0 to about 1.25 mg KOH/gram, or about 1.1 to about 1.2 mg KOH/gram.

Preferably, the boronated and the non-boronated oil-soluble nitrogen-containing compounds of the dispersant system herein are polyisobutylene succinimide dispersants derived from a polyisobutylene having a number average molecular weight of at least about 350 and, preferably, polyisobutylene succinimide dispersants derived from polyisobutylene having a number average molecular weight of about 1,000 to about 5,000; about 1,200 to about 3,000; or about 1,200 to about 2,600. In one approach, the dispersant system herein includes a blend of (i) at least one boronated polyisobutylene succinimide dispersant derived from polyisobutylene having a number average molecular weight less than 2,000 and, preferably about 1,000 to about 1,800, and (ii) at least one non-boronated polyisobutylene succinimide dispersant derived from polyisobutylene having a number average molecular weight greater than 2,000 and, preferably, about 2,000 to about 3,000.

Oil soluble nitrogen-containing dispersants are often known as ashless-type dispersants because, prior to mixing in a lubricating composition, they do not contain ash-forming metals and they do not normally contribute any ash when added to a lubricant. Ashless type dispersants are characterized by a polar group attached to a relatively high molecular weight hydrocarbon chain. Typical ashless dispersants include N-substituted long chain alkenyl succinimides. Examples of nitrogen-substituted long chain alkenyl succinimides include polyisobutylene succinimide with the number average molecular weight of the polyisobutylene substituent being in the range about 350 to about 50,000, or to about 5,000, or to about 3,000, or to about 2,000 to about 3,000 as measured by GPC. As mentioned above, the molecular weight of the polyisobutylene substituent may vary depending on whether the dispersant is boronated or non-boronated. Succinimide dispersants and their preparation are disclosed, for instance in U.S. Pat. No. 7,897,696 or U.S. Pat. No. 4,234,435, which are incorporated herein by reference. The alkenyl substituent may be prepared from polymerizable monomers containing about 2 to about 16, or about 2 to about 8, or about 2 to about 6 carbon atoms. Succinimide dispersants are typically the imide formed from a polyamine, typically a poly(ethyleneamine).

In approaches, preferred amines for the dispersants may be selected from polyamines and hydroxylamines. Examples of polyamines that may be used include, but are not limited to, diethylene triamine (DETA), triethylene tetramine (TETA), tetraethylene pentamine (TEPA), and higher homologues such as pentaethylene hexamine (PEHA), and the like. In some approaches, a so-called heavy polyamine may be used, which is a mixture of polyalkylene-polyamines comprising small amounts of lower polyamine oligomers such as TEPA and PEHA (pentaethylene hexamine) but primarily oligomers with 6 or more nitrogen atoms, 2 or more primary amines per molecule, and more extensive branching than conventional polyamine mixtures. A heavy polyamine preferably includes polyamine oligomers containing 7 or more nitrogen atoms per molecule and with 2 or more primary amines per molecule.

In some embodiments, polyisobutylene (PIB), when included, is a preferred reactant to form the dispersants and may have greater than 50 mol %, greater than 60 mol %, greater than 70 mol %, greater than 80 mol %, or greater than 90 mol % content of terminal double bonds. Such PIB is also referred to as highly reactive PIB ("HR-PIB"). HR-PIB having a number average molecular weight ranging from about 800 to about 5000, as determined by GPC, is suitable for use in embodiments of the present disclosure. Conventional PIB typically has less than 50 mol %, less than 40 mol %, less than 30 mol %, less than 20 mol %, or less than 10 mol % content of terminal double bonds.

An HR-PIB having a number average molecular weight ranging from about 900 to about 3,000 may be suitable, as determined by GPC or, preferably about 2,000 to about 3,000. Such HR-PIB is commercially available, or can be synthesized by the polymerization of isobutene in the presence of a non-chlorinated catalyst such as boron trifluoride, as described in U.S. Pat. No. 4,152,499 and/or U.S. Pat. No. 5,739,355. When used in the aforementioned thermal ene reaction, HR-PIB may lead to higher conversion rates in the reaction, as well as lower amounts of sediment formation, due to increased reactivity. A suitable method is described in U.S. Pat. No. 7,897,696. In one embodiment, the present disclosure further comprises at least one dispersant derived from polyisobutylene succinic anhydride ("PIBSA"). The PIBSA may have an average of between about 1.0 and about 2.0 succinic acid moieties per polymer.

As mentioned above, the dispersant system herein includes a blend of post treated and non-post treated dispersants. For instance, some of the dispersants herein may be free of any post-treatments, such as post treatments with boron, urea, thiourea, dimercapto thiadiazoles, carbon disulfide, aldehydes, ketones, carboxylic acids, hydrocarbon-substituted succinic anhydrides, maleic anhydride, nitriles, epoxides, carbonates, cyclic carbonates, hindered phenolic esters, and phosphorus compound. Other dispersants may be post-treated by conventional methods by a reaction with any of a variety of agents. Suitable post treat agents include boron, urea, thiourea, dimercapto thiadiazoles, carbon disulfide, aldehydes, ketones, carboxylic acids, hydrocarbon-substituted succinic anhydrides, maleic anhydride, nitriles, epoxides, carbonates, cyclic carbonates, hindered phenolic esters, and phosphorus compounds. (See, e.g., U.S. Pat. Nos. 7,645,726; 7,214,649; 8,048,831; and 5,241,003, which are all incorporated herein by reference in their entireties.) Preferably, at least one of the dispersants in the dispersant systems herein is post treated with a boron compound.

When post treated with boron, the boron compound used as a post-treating reagent can be selected from boron oxide, boron halides, boron acids and esters of boron acids in an amount to provide from about 0.1 atomic proportion of boron for each mole of the nitrogen composition to about 20 atomic proportions of boron for each atomic proportion of nitrogen used. The dispersant post-treated with boron may contain from about 0.05 weight percent to about 2.0 weight percent, or in other approaches, about 0.05 weight percent to about 0.7 weight percent boron, based on the total weight of the borated dispersant.

In other approaches and if used, a carboxylic acid post treat agent may optionally be used with either the boronated or the non-boronated dispersants herein and can be saturated or unsaturated mono-, di-, or poly-carboxylic acid. Examples of carboxylic acids include, but are not limited to, maleic acid, fumaric acid, succinic acid, and naphthalic diacid (e.g., 1,8-naphthalic diacid). Anhydrides can also be used as a post-treating reagent and can be selected from the

group consisting of mono-unsaturated anhydride (e.g., maleic anhydride), alkyl or alkylene-substituted cyclic anhydrides (e.g., succinic anhydride or glutamic anhydride), and aromatic carboxylic anhydrides (including naphthalic anhydride, e.g., 1,8-naphthalic anhydride).

In one embodiment and if used, the process of post-treating the dispersant includes first forming the succinimide product, as described above, and then further reacting the succinimide product with the post treating agent, such as a boron compound, such as boric acid. In some cases, the dispersants herein may be post-treated with more than one post-treatment agents. For example, the dispersant may be post-treated with a boron compound, such as boric acid, and also an anhydride, such as maleic anhydride and/or 1,8-naphthalic anhydride.

In embodiments, the passenger car motor oil lubricating combinations herein may include up to about 10 weight percent of individual or combined dispersant additives, in other approaches, about 0.1 to about 8 weight percent, about 0.2 to about 6 weight percent, or about 0.2 to about 5 weight percent of individual or total dispersant additives. In some embodiments, the dispersant systems herein may have more of the non-boronated dispersants than the boronated dispersants, and may have a weight ratio of dispersant boron to dispersant nitrogen of less than 0.3:1, less than about 0.28:1, or less than about 0.25:1. In other approaches, the dispersant system may have a weight ratio of the dispersant boron to the dispersant nitrogen of about 0.15:1 to 0.3:1, about 0.18:1 to about 0.28:1, or about 0.2:1 to about 0.25:1.

#### The Detergent System

The passenger car motor oil lubricating compositions herein also include a detergent system with one or more metal-containing detergent additives providing at least about 0.25 weight percent soap to the lubricant. In one approach, the detergent system includes metal-containing detergent additives of (i) at least one calcium-containing detergent additive providing an amount of calcium soap to the lubricant and (ii) at least one magnesium-containing detergent additive providing an amount of magnesium soap to the lubricant. In some approaches, the detergent system provides more of the calcium soap than the magnesium soap to the passenger car motor oil lubricating composition. In other approaches, the metal containing detergent additives herein may have a weight ratio of the calcium soap to the magnesium soap of up to about 1:6:1, in other approaches, up to about 1.4:1, or about 1.1:1 to about 1.6:1 or about 1.2:1 to about 1.4:1.

In some approaches, the detergent systems herein to are substantially free of metal-containing phenate detergents and, thus, the detergent systems herein are substantially free of or do not provide any phenate soap to the lubricants. As used herein, substantially free of generally means about 0.1 weight percent or less, about 0.05 weight percent or less, about 0.01 weight percent or less, or no functional amounts of phenate detergents or phenate soaps.

In one approach or embodiment, the one or more detergent additives include a calcium-containing detergent additive, and more preferably a sulfonate-based, calcium-providing detergent. The one or more detergent additives may also include a magnesium-containing detergent additive, and more preferably, a sulfonate-based, magnesium detergent additive. These select detergent additives have a total base number (TBN) of at least about 3 mg KOH/g, at least about 4 mg KOH/g, at least about 5 mg KOH/g, or at least about 6 mg KOH/g as measured pursuant to ASTM D2896, and in

other approaches or embodiments, the detergents herein provide a TBN of about 10 mg KOH/g or less to the lubricants.

Suitable detergents and their methods of preparation are described in greater detail in numerous patent publications, including U.S. Pat. No. 7,732,390 and references cited therein, which are incorporated herein by reference. The passenger car motor oil lubricating compositions herein may include about 0.1 to about 5 weight percent of individual and/or total detergent additives, and in other approaches, about 0.15 to about 3 weight percent, and in yet other approaches, about 0.15 to 2.6 weight percent of individual and/or total detergent additives so long as the detergent additives meet the calcium, magnesium, and/or soap contents noted herein.

Generally, suitable detergents in the lubricants herein (subject to the noted requirements of calcium, magnesium, and soap contents herein) may include linear or branched alkali or alkaline earth metal salts, such as calcium, sodium, or magnesium, of petroleum sulfonic acids and long chain mono- or di-alkylaryl sulfonic acids with the aryl group being benzyl, tolyl, and xylol and/or various phenates or derivatives of phenates. Examples of suitable detergents include, subject the required amounts of sulfonate soap noted above, low-based/neutral and overbased variations of the following detergents: calcium phenates, calcium sulfur containing phenates, calcium sulfonates, calcium calixarates, calcium salixarates, calcium salicylates, calcium carboxylic acids, calcium phosphorus acids, calcium mono- and/or di-thiophosphoric acids, calcium alkyl phenols, calcium sulfur coupled alkyl phenol compounds, calcium methylene bridged phenols, magnesium phenates, magnesium sulfur containing phenates, magnesium sulfonates, magnesium calixarates, magnesium salixarates, magnesium salicylates, magnesium carboxylic acids, magnesium phosphorus acids, magnesium mono- and/or di-thiophosphoric acids, magnesium alkyl phenols, magnesium sulfur coupled alkyl phenol compounds, magnesium methylene bridged phenols, sodium phenates, sodium sulfur containing phenates, sodium sulfonates, sodium calixarates, sodium salixarates, sodium salicylates, sodium carboxylic acids, sodium phosphorus acids, sodium mono- and/or di-thiophosphoric acids, sodium alkyl phenols, sodium sulfur coupled alkyl phenol compounds, or sodium methylene bridged phenols.

As understood, overbased detergent additives are well-known in the art and may be alkali or alkaline earth metal overbased detergent additives. Such detergent additives may be prepared by reacting a metal oxide or metal hydroxide with a substrate and carbon dioxide gas. The substrate is typically an acid, for example, an acid such as an aliphatic substituted sulfonic acid, an aliphatic substituted carboxylic acid, or an aliphatic substituted phenol.

The term "overbased" relates to metal salts, such as metal salts of sulfonates, carboxylates, salicylates and/or phenates, wherein the amount of metal present exceeds the stoichiometric amount. Such salts may have a conversion level in excess of 100% (i.e., they may comprise more than 100% of the theoretical amount of metal needed to convert the acid to its "normal," "neutral" salt). The expression "metal ratio," often abbreviated as MR, is used to designate the ratio of total chemical equivalents of metal in the overbased salt to chemical equivalents of the metal in a neutral salt according to known chemical reactivity and stoichiometry. In a normal or neutral salt, the MR is one and in an overbased salt, MR, is greater than one. They are commonly referred to as overbased, hyperbased, or superbased salts and may be salts of organic sulfur acids, carboxylic acids, or phenols.

As used herein, the term "TBN" is used to denote the Total Base Number in mg KOH/g as measured by the method of ASTM D2896. The detergent may be neutral or overbased. For example, a low-base or neutral detergent herein may have a total base number (TBN) of up to about 250 mg KOH/gram as noted above. Overbased detergents, which may be provided in the passenger car motor oil and/or the finished lubricants herein, may have a total base number (TBN) of about 250 mg KOH/gram or greater, or about 300 mg KOH/gram or greater, or about 350 mg KOH/gram or greater, or about 375 mg KOH/gram or greater, or about 400 mg KOH/gram or greater. The overbased detergent may have a metal to substrate ratio of from 1.1:1 or less, or from 2:1 or less, or from 4:1 or less, or from 5:1 or less, or from 7:1 or less, or from 10:1 or less, or from 12:1 or less, or from 15:1 or less, or from 20:1 or less.

Examples of suitable overbased detergents include, but are not limited to, overbased calcium phenates, overbased calcium sulfur containing phenates, overbased calcium sulfonates, overbased calcium calixarates, overbased calcium salixarates, overbased calcium salicylates, overbased calcium carboxylic acids, overbased calcium phosphorus acids, overbased calcium mono- and/or di-thiophosphoric acids, overbased calcium alkyl phenols, overbased calcium sulfur coupled alkyl phenol compounds, overbased calcium methylene bridged phenols, overbased magnesium phenates, overbased magnesium sulfur containing phenates, overbased magnesium sulfonates, overbased magnesium calixarates, overbased magnesium salixarates, overbased magnesium salicylates, overbased magnesium carboxylic acids, overbased magnesium phosphorus acids, overbased magnesium mono- and/or di-thiophosphoric acids, overbased magnesium alkyl phenols, overbased magnesium sulfur coupled alkyl phenol compounds, or overbased magnesium methylene bridged phenols. Preferably, the detergents are magnesium sulfonate and calcium sulfonate and, as mentioned above, substantially free of phenate detergents. More preferably, the detergents herein are overbased magnesium sulfonate and overbased calcium sulfonate.

In other embodiments, the TBN of the detergents herein may reflect a neat or non-diluted version of the detergent component. For example, the fluids herein may include overbased calcium sulfonate or an overbased magnesium sulfonate, as a neat additive, having a TBN of about 300 to about 450, and in other approaches, about 380 to about 420.

In some approaches or embodiments, the detergent systems herein provide at least about 0.25 weight percent soap to the lubricant, and more preferably, about 0.25 weight percent soap to about 0.4 weight percent soap. In approaches, the soap content is about 50 to about 60 percent calcium-based soap and about 40 to about 60 percent magnesium based soap. In other approaches, the metal containing detergent additives herein may have a weight ratio of the calcium soap to the magnesium soap of up to about 1:6:1, in other approaches, up to about 1.4:1, or about 1.1:1 to about 1.6:1 or about 1.2:1 to about 1.4:1.

Soap content generally refers to the amount of neutral organic acid salt and reflects a detergent's cleansing ability, or detergency, and dirt suspending ability. The soap content of a lubricant can be determined by ASTM D3712. Further discussion on determining soap content can be found in FUELS AND LUBRICANTS HANDBOOK, TECHNOLOGY, PROPERTIES, PERFORMANCE, AND TESTING, George Totten, editor, ASTM International, 2003, relevant portions thereof incorporated herein by reference.

#### Viscosity Index Improver

The passenger car motor oil lubricating oil compositions herein may optionally contain one or more viscosity index improvers. Preferably, any viscosity index improver, if used, has a shear stability index (SSI) of less than about 50 as measured pursuant to ASTM D6278. In other approaches, the viscosity index improves of the compositions herein when used have a SSI of about 40 or less, about 35 or less, or about 30 or less and, in some approaches, have a SSI of about 25 to about 50, about 25 to about 40, or about 25 to about 25.

Suitable viscosity index improvers may include polyolefins, olefin copolymers, ethylene/propylene copolymers, polyisobutenes, hydrogenated styrene-isoprene polymers, styrene/maleic ester copolymers, hydrogenated styrene/butadiene copolymers, hydrogenated isoprene polymers, alpha-olefin maleic anhydride copolymers, polymethacrylates, polyacrylates, polyalkyl styrenes, hydrogenated alk-  
enyl aryl conjugated diene copolymers, or mixtures thereof.

Viscosity index improvers may include star polymers and suitable examples are described in US 2012/0101017A1.

Preferably, the viscosity index improver is a non-dispersant viscosity index improver; however, the lubricating oil compositions herein also may optionally contain one or more dispersant viscosity index improvers in addition to a non-dispersant viscosity index improver. Suitable viscosity index improvers may include functionalized polyolefins, for example, ethylene-propylene copolymers that have been functionalized with the reaction product of an acylating agent (such as maleic anhydride) and an amine; polymethacrylates functionalized with an amine, or esterified maleic anhydride-styrene copolymers reacted with an amine.

The total amount of viscosity index improver and/or dispersant viscosity index improver may be about 0 weight percent to about 20 weight percent, about 0.1 wt weight percent to about 15 weight percent, about 0.1 weight percent to about 12 weight percent, or about 0.5 weight percent to about 10 weight percent, of the passenger car motor oil lubricating compositions herein.

#### 40 Metal Dihydrocarbyl Dithiophosphate Compounds

The passenger car motor oil lubricating compositions herein may optionally include one or more metal dihydrocarbyl dithiophosphate compounds, such as but not limited to, a zinc dihydrocarbyl dithiophosphate compound (ZDDP). If used, the one or more metal dihydrocarbyl dithiophosphate compounds may provide up to about 1,000 ppm phosphorus to the lubricant, up to about 900 ppm phosphorus, or up to about 800 phosphorus to the lubricant package or at least about 200 ppm of phosphorus. When used in the lubricants herein, the hydrocarbyl groups of the one or more metal dihydrocarbyl dithiophosphate compounds are preferably derived from a mixture of secondary alcohols and primary alcohols and with a ratio of the primary alcohols to the secondary alcohols of about 0.3:1 to about 0.6:1. In other approaches, the average number of carbon atoms in the hydrocarbyl groups per primary alcohol may be no more than about 0.6:1, and preferably, about 0.3:1 to about 0.6:1.

Suitable metal dihydrocarbyl dithiophosphates compounds may include between 5 to about 10 weight percent metal (such as, about 6 to about 9 weight percent metal such as zinc), and about 8 to about 18 weight percent sulfur, (such as about 12 to about 18 weight percent sulfur, or about 8 to about 15 weight percent sulfur). Suitable metal dihydrocarbyl dithiophosphate compounds may comprise dihydrocarbyl dithiophosphate metal salts wherein the metal may be an alkali metal, alkaline earth metal, aluminum, lead, tin,

molybdenum, manganese, nickel, copper, titanium, zirconium, zinc, or combinations thereof. Preferably, the metal is zinc.

The alkyl groups on the metal dihydrocarbyl dithiophosphate compounds when used in the passenger car motor oil herein may be derived from primary alcohols, secondary alcohols, phenols, and preferably, is derived from a mixture of primary and secondary alcohols. For example, the hydrocarbyl groups may be derived from a mixture of primary and secondary alcohols including 2-ethyl hexanol, methyl isobutyl carbinol (MIBC), isobutanol, and isopropanol. For example, about 60 mol percent or more of the alkyl groups may be derived from primary alcohols (such as, but not limited to, 2-ethyl hexanol and/or isobutyl alcohol) and about 40 mol percent or less of alkyl groups may be derived from secondary alcohols (such as, but not limited to, isopropyl alcohol, methyl isobutyl carbinol, and the like, and/or combinations thereof). In optional approaches, all of the alkyl groups on the metal dihydrocarbyl dithiophosphate compounds may be derived from a primary alcohol, such as 2-ethyl hexanol or others noted below. In other optional approaches, all of the alkyl groups on the metal dihydrocarbyl dithiophosphate compounds may be derived from a secondary alcohol, such as, but not limited to isopropyl alcohol, or methyl isobutyl carbinol.

In one approach, the metal dihydrocarbyl dithiophosphate compound of the lubricants herein may be a blend of two ZDDP compounds including about 40 to about 60 mol percent of ethyl hexanol and about 40 to about 60 mol percent of methyl isobutyl carbinol and may include about 6 to about 10 weight percent phosphorus, about 6 to about 9 weight percent zinc, and about 12 to about 18 weight percent sulfur. In another approach, the metal dihydrocarbyl dithiophosphate compound of the passenger car motor oil may be one or more ZDDP compounds obtained from 80 to 100 mol percent of 2-ethyl hexyl alcohol or 80 to 100 mol percent of methyl isobutyl carbinol and may include about 6 to about 10 weight percent phosphorus, about 6 to about 9 weight percent zinc, and about 12 to about 18 weight percent sulfur. Most preferably, the ZDDP compounds herein is a blend of ZDDP compounds with one having 100 mol percent of primary alcohols and the other having 100 mol percent of secondary alcohols.

In general, subject to the limitations noted above, the metal dihydrocarbyl dithiophosphate compounds of the passenger car motor oil may be derived from, but not limited to, alcohols selected from 2-ethylhexanol, methylheptanol, heptanol, octanol, nonanol, decanol, dodecanol, and/or isovalinvariants thereof. Examples of suitable metal dihydrocarbyl dithiophosphate compounds include, but are not limited, to: zinc O,O-di(C<sub>8-14</sub>-alkyl)dithiophosphate; zinc O,O-bis(2-ethylhexyl) dithiophosphate; zinc O,O-diisooctyl dithiophosphate; zinc O,O-bis(dodecylphenyl) dithiophosphate; zinc O,O-diisodecyl dithiophosphate; zinc O,O-bis(6-methylheptyl) dithiophosphate; zinc O,O-dioctyl dithiophosphate; zinc O,O-dipentyl dithiophosphate; zinc O-(2-methylbutyl)-O-(2-methylpropyl)dithiophosphate; and zinc O-(3-methylbutyl)-O-(2-methylpropyl) dithiophosphate, or combinations thereof.

In approaches or embodiments, the metal dihydrocarbyl dithiophosphate compound suitable for the passenger car motor oils herein may have a structure of Formula I:

(Formula I)



wherein each R in Formula I independently contains from 6 to 18 carbon atoms, or 6 to 12 carbon atoms, or about 8 to 10 carbon atoms so long as each phosphorus atom has, on average, at least 14 total carbons, and preferably at least 8 total carbons or 8 to 16 total carbons per phosphorus atom. For example, each R may independently be ethyl, n-propyl, i-propyl, n-butyl, i-butyl, sec-butyl, amyl, n-hexyl, i-hexyl, n-octyl, decyl, dodecyl, octadecyl, 2-ethylhexyl, phenyl, butylphenyl, cyclohexyl, methylcyclopentyl, propenyl, butenyl. The number of carbon atoms in each R group in the formula above will generally be about 3 or greater, about 4 or greater, about 6 or greater, or about 8 or greater. Each R group may average 6 to 10 carbons and, preferably 8 to 10 carbons. Preferably, each R may be linear or branched C8 or 2-ethylhexyl groups, C3 or isopropyl groups, and/or C4 or isobutyl groups. In Formula I, A is a metal, such as aluminum, lead, tin, molybdenum, manganese, nickel, copper, titanium, zirconium, zinc, or combinations thereof and, preferably, A is zinc. When the metal dihydrocarbyl dithiophosphate compound has the structure shown in Formula I and with A being zinc, the compound may have about 4 to about 9 weight percent phosphorus and about 6 to about 9 weight percent zinc and a zinc to phosphorus ratio of about 1.0 to about 1.5.

In some approaches or embodiments, it is understood in the art that a more accurate representation of the sulfur-zinc coordination arrangement may be represented by the symmetrical arrangement shown below with the chemical structure of Formula II that may be used herein as interchangeable with Formula I shown above. It is also understood that the structures shown in Formulas I and II may be present as monomer, dimer, trimer, or oligomer (such as a tetramer).



(Formula II)

Dihydrocarbyl dithiophosphate metal salts may be prepared in accordance with known techniques by first forming a dihydrocarbyl dithiophosphoric acid (DDPA), usually by reaction of one or more alcohols or phenols with P<sub>2</sub>S<sub>5</sub> and then neutralizing the formed DDPA with a metal compound, such as zinc oxide. For example, DDPA may be made by reacting mixtures of alcohols including the suitable amounts of primary alcohols (and if needed, suitable blends of primary and secondary alcohols) with P<sub>2</sub>S<sub>5</sub>. In this case, the DDPA includes alkyl groups predominately derived from primary alcohols or both primary and secondary alcohols as needed to meet the required primary alcohol content in the final product. Alternatively, multiple DDPA's can be prepared where the alkyl groups on one DDPA are derived entirely from secondary alcohols and the alkyl groups on another DDPA are derived entirely from primary alcohols. The DDPA's are then blended together to form a mixture of DDPA's having alkyl groups meeting the noted primary alcohol content.

As mentioned, the passenger car motor oil may include blends of metal dihydrocarbyl dithiophosphate compounds derived from primary alcohols and/or secondary alcohols. In one approach, the finished lubricants herein may include about 1 to about 5 weight percent of the metal dihydrocarbyl dithiophosphate compounds.

Base Oil or Base Oil Blend:

As discussed above, a base oil herein may be oils of lubricating viscosity and selected from any of the base oils in API Groups I to V as specified in the American Petroleum Institute (API) Base Oil Interchangeability Guidelines and, preferably, is a blend of one or more API Group II base oils combined with API Group III and/or Group IV base oils. More preferably, the base oil is a blend having at least about 25 weight percent of API Group II base oil, at least about 50 weight percent of API Group II base oils or, alternatively, a blend of about 25 to about 80 weight percent of API Group II base oils combined with about 20 to about 75 weight percent of API Group III base oils. In some embodiments, the base oil systems herein, in some approaches or embodiments, including the blend of Group II and Group III and/or Group IV base oils may have a KV100 of about 2 to about 20 cSt, in other approaches, about 5 to about 15 cSt, about 8 to about 15 cSt, in yet other approaches, about 10 to about 15 cSt. As known, the five base oil groups are generally set forth in Table 1 below:

TABLE 1

| Base oil Category | Sulfur (%)                                          | Saturates (%) | Viscosity Index |
|-------------------|-----------------------------------------------------|---------------|-----------------|
| Group I           | >0.03                                               | and/or        | <90 80 to 120   |
| Group II          | ≤0.03                                               | and           | ≥90 80 to 120   |
| Group III         | ≤0.03                                               | and           | ≥90 ≥120        |
| Group IV          | All polyalphaolefins (PAOs)                         |               |                 |
| Group V           | All others not included in Groups I, II, III, or IV |               |                 |

Groups I, II, and III are mineral oil process stocks. Group IV base oils contain true synthetic molecular species, which are produced by polymerization of olefinically unsaturated hydrocarbons. Many Group V base oils are also true synthetic products and may include diesters, polyol esters, polyalkylene glycols, alkylated aromatics, polyphosphate esters, polyvinyl ethers, and/or polyphenyl ethers, and the like, but may also be naturally occurring oils, such as vegetable oils. It should be noted that although Group III base oils are derived from mineral oil, the rigorous processing that these fluids undergo causes their physical properties to be very similar to some true synthetics, such as PAOs. Therefore, oils derived from Group III base oils may be referred to as synthetic fluids in the industry. Group II+ may comprise high viscosity index Group II.

The base oil blend used in the disclosed lubricating oil composition may be a mineral oil, animal oil, vegetable oil, synthetic oil, synthetic oil blends, or mixtures thereof. Suitable oils may be derived from hydrocracking, hydrogenation, hydrofinishing, unrefined, refined, and re-refined oils, and mixtures thereof.

Unrefined oils are those derived from a natural, mineral, or synthetic source without or with little further purification treatment. Refined oils are similar to the unrefined oils except that they have been treated in one or more purification steps, which may result in the improvement of one or more properties. Examples of suitable purification techniques are solvent extraction, secondary distillation, acid or base extraction, filtration, percolation, and the like. Oils

refined to the quality of an edible may or may not be useful. Edible oils may also be called white oils. In some embodiments, lubricating oil compositions are free of edible or white oils.

5 Re-refined oils are also known as reclaimed or reprocessed oils. These oils are obtained similarly to refined oils using the same or similar processes. Often these oils are additionally processed by techniques directed to removal of spent additives and oil breakdown products.

10 Mineral oils may include oils obtained by drilling or from plants and animals or any mixtures thereof. For example such oils may include, but are not limited to, castor oil, lard oil, olive oil, peanut oil, corn oil, soybean oil, and linseed oil, as well as mineral lubricating oils, such as liquid petroleum oils and solvent-treated or acid-treated mineral lubricating oils of the paraffinic, naphthenic or mixed paraffinic-naphthenic types. Such oils may be partially or fully hydrogenated, if desired. Oils derived from coal or shale may also be useful.

15 Useful synthetic lubricating oils may include hydrocarbon oils such as polymerized, oligomerized, or interpolymerized olefins (e.g., polybutylenes, polypropylenes, propyleneisobutylene copolymers); poly(1-hexenes), poly(1-octenes), trimers or oligomers of 1-decene, e.g., poly(1-decenes), such materials being often referred to as  $\alpha$ -olefins, and mixtures thereof; alkyl-benzenes (e.g. dodecylbenzenes, tetradecylbenzenes, dinonylbenzenes, di-(2-ethylhexyl)-benzenes); polyphenyls (e.g., biphenyls, terphenyls, alkylated polyphenyls); diphenyl alkanes, alkylated diphenyl alkanes, alkylated diphenyl ethers and alkylated diphenyl sulfides and the derivatives, analogs and homologs thereof or mixtures thereof. Polyalphaolefins are typically hydrogenated materials.

20 Other synthetic lubricating oils include polyol esters, diesters, liquid esters of phosphorus-containing acids (e.g., tricresyl phosphate, trioctyl phosphate, and the diethyl ester of decane phosphonic acid), or polymeric tetrahydrofurans. Synthetic oils may be produced by Fischer-Tropsch reactions and typically may be hydroisomerized Fischer-Tropsch hydrocarbons or waxes. In one embodiment oils may be prepared by a Fischer-Tropsch gas-to-liquid synthetic procedure as well as other gas-to-liquid oils.

25 The major amount of base oil included in a lubricating 45 composition may be selected from the group consisting of Group I, Group II, a Group III, a Group IV, a Group V, and a combination of two or more of the foregoing, and wherein the major amount of base oil is other than base oils that arise from provision of additive components or viscosity index improvers in the composition. In another embodiment, the major amount of base oil included in a lubricating composition may be selected from the group consisting of Group II, a Group III, a Group IV, a Group V, and a combination of two or more of the foregoing, and wherein the major 50 amount of base oil is other than base oils that arise from provision of additive components or viscosity index improvers in the composition.

30 The amount of the oil of lubricating viscosity present may be the balance remaining after subtracting from 100 wt % 60 the sum of the amount of the performance additives inclusive of viscosity index improver(s) and/or pour point depressant(s) and/or other top treat additives. For example, the oil of lubricating viscosity that may be present in a finished fluid may be a major amount, such as greater than about 50 wt %, greater than about 60 wt %, greater than about 70 wt %, greater than about 80 wt %, greater than about 85 wt %, or greater than about 90 wt %.

As generally used herein, the terms "oil composition," "lubrication composition," "lubricating oil composition," "lubricating oil," "lubricant composition," "lubricant," and "lubricating" are considered synonymous, fully interchangeable terminology referring to a passenger car motor oil lubrication product comprising a major amount of a base oil component having the blend amounts noted above plus minor amounts of the detergents and the other optional components that is preferably API GF-6 capable.

Optional Additives:

The passenger car motor oil lubricating compositions herein may also include a number of optional additives combined with the detergent systems and dispersant system discussed above and as needed to meet performance standards. Those optional additives are described in the following paragraphs.

Other Dispersants: The lubricating oil composition may optionally include one or more other dispersants or mixtures thereof. Dispersants are often known as ashless-type dispersants because, prior to mixing in a lubricating oil composition, they do not contain ash-forming metals and they do not normally contribute any ash when added to a lubricant. Ashless type dispersants are characterized by a polar group attached to a relatively high molecular weight hydrocarbon chain. Typical ashless dispersants include N-substituted long chain alkenyl succinimides. Examples of N-substituted long chain alkenyl succinimides include polyisobutylene succinimide with the number average molecular weight of the polyisobutylene substituent being in the range about 350 to about 50,000, or to about 5,000, or to about 3,000, as measured by GPC. Succinimide dispersants and their preparation are disclosed, for instance in U.S. Pat. No. 7,897,696 or U.S. Pat. No. 4,234,435. The alkenyl substituent may be prepared from polymerizable monomers containing about 2 to about 16, or about 2 to about 8, or about 2 to about 6 carbon atoms. Succinimide dispersants are typically the imide formed from a polyamine, typically a poly(ethyl-eneamine).

Preferred amines are selected from polyamines and hydroxylamines. Examples of polyamines that may be used include, but are not limited to, diethylene triamine (DETA), triethylene tetramine (TETA), tetraethylene pentamine (TEPA), and higher homologues such as pentaethylene hexamine (PEHA), and the like.

A suitable heavy polyamine is a mixture of polyalkylene-polyamines comprising small amounts of lower polyamine oligomers such as TEPA and PEHA (pentaethylene hexamine) but primarily oligomers with 6 or more nitrogen atoms, 2 or more primary amines per molecule, and more extensive branching than conventional polyamine mixtures. A heavy polyamine preferably includes polyamine oligomers containing 7 or more nitrogen atoms per molecule and with 2 or more primary amines per molecule. The heavy polyamine comprises more than 28 wt. % (e.g. >32 wt. %) total nitrogen and an equivalent weight of primary amine groups of 120-160 grams per equivalent.

In some approaches, suitable polyamines are commonly known as PAM and contain a mixture of ethylene amines where TEPA and pentaethylene hexamine (PEHA) are the major part of the polyamine, usually less than about 80%.

Typically, PAM has 8.7-8.9 milliequivalents of primary amine per gram (an equivalent weight of 115 to 112 grams per equivalent of primary amine) and a total nitrogen content of about 33-34 wt. %. Heavier cuts of PAM oligomers with practically no TEPA and only very small amounts of PEHA but containing primarily oligomers with more than 6 nitro-

gen atoms and more extensive branching, may produce dispersants with improved dispersancy.

In an embodiment the present disclosure further comprises at least one polyisobutylene succinimide dispersant derived from polyisobutylene with a number average molecular weight in the range about 350 to about 50,000, or to about 5000, or to about 3000, as determined by GPC. The polyisobutylene succinimide may be used alone or in combination with other dispersants.

10 In some embodiments, polyisobutylene, when included, may have greater than 50 mol %, greater than 60 mol %, greater than 70 mol %, greater than 80 mol %, or greater than 90 mol % content of terminal double bonds. Such PIB is also referred to as highly reactive PIB ("HR-PIB"). HR-PIB 15 having a number average molecular weight ranging from about 800 to about 5000, as determined by GPC, is suitable for use in embodiments of the present disclosure. Conventional PIB typically has less than 50 mol %, less than 40 mol %, less than 30 mol %, less than 20 mol %, or less than 10 mol % content of terminal double bonds.

An HR-PIB having a number average molecular weight ranging from about 900 to about 3000 may be suitable, as determined by GPC. Such HR-PIB is commercially available, or can be synthesized by the polymerization of 25 isobutene in the presence of a non-chlorinated catalyst such as boron trifluoride, as described in U.S. Pat. No. 4,152,499 to Boerzel, et al. and U.S. Pat. No. 5,739,355 to Gateau, et al. When used in the aforementioned thermal ene reaction, HR-PIB may lead to higher conversion rates in the reaction, 30 as well as lower amounts of sediment formation, due to increased reactivity. A suitable method is described in U.S. Pat. No. 7,897,696.

In one embodiment, the present disclosure further comprises at least one dispersant derived from polyisobutylene 35 succinic anhydride ("PIBSA"). The PIBSA may have an average of between about 1.0 and about 2.0 succinic acid moieties per polymer.

The % actives of the alkenyl or alkyl succinic anhydride can be determined using a chromatographic technique. This 40 method is described in column 5 and 6 in U.S. Pat. No. 5,334,321.

The percent conversion of the polyolefin is calculated from the % actives using the equation in column 5 and 6 in U.S. Pat. No. 5,334,321.

45 Unless stated otherwise, all percentages are in weight percent and all molecular weights are number average molecular weights determined by gel permeation chromatography (GPC) using commercially available polystyrene standards (with a number average molecular weight of 180 to about 18,000 as the calibration reference).

In one embodiment, the dispersant may be derived from a polyalphaolefin (PAO) succinic anhydride. In one embodiment, the dispersant may be derived from olefin maleic anhydride copolymer. As an example, the dispersant may be 55 described as a poly-PIBSA. In an embodiment, the dispersant may be derived from an anhydride which is grafted to an ethylene-propylene copolymer.

A suitable class of nitrogen-containing dispersants may be derived from olefin copolymers (OCP), more specifically, 60 ethylene-propylene dispersants which may be grafted with maleic anhydride. A more complete list of nitrogen-containing compounds that can be reacted with the functionalized OCP are described in U.S. Pat. Nos. 7,485,603; 7,786,057; 7,253,231; 6,107,257; and 5,075,383; and/or are commercially available.

65 One class of suitable dispersants may also be Mannich bases. Mannich bases are materials that are formed by the

condensation of a higher molecular weight, alkyl substituted phenol, a polyalkylene polyamine, and an aldehyde such as formaldehyde. Mannich bases are described in more detail in U.S. Pat. No. 3,634,515.

A suitable class of dispersants may also be high molecular weight esters or half ester amides. A suitable dispersant may also be post-treated by conventional methods by a reaction with any of a variety of agents. Among these are boron, urea, thiourea, dimercaptothiadiazoles, carbon disulfide, aldehydes, ketones, carboxylic acids, hydrocarbon-substituted succinic anhydrides, maleic anhydride, nitriles, epoxides, carbonates, cyclic carbonates, hindered phenolic esters, and phosphorus compounds. U.S. Pat. Nos. 7,645,726; 7,214,649; and 8,048,831 are incorporated herein by reference in their entireties.

In addition to the carbonate and boric acids post-treatments both the compounds may be post-treated, or further post-treatment, with a variety of post-treatments designed to improve or impart different properties. Such post-treatments include those summarized in columns 27-29 of U.S. Pat. No. 5,241,003, hereby incorporated by reference. Such treatments include, treatment with: Inorganic phosphorous acids or anhydrides (e.g., U.S. Pat. Nos. 3,403,102 and 4,648,980); Organic phosphorous compounds (e.g., U.S. Pat. No. 3,502,677); Phosphorous pentasulfides; Boron compounds as already noted above (e.g., U.S. Pat. Nos. 3,178,663 and 4,652,387); Carboxylic acid, polycarboxylic acids, anhydrides and/or acid halides (e.g., U.S. Pat. Nos. 3,708,522 and 4,948,386); Epoxides polyepoxides or thioepoxides (e.g., U.S. Pat. Nos. 3,859,318 and 5,026,495); Aldehyde or ketone (e.g., U.S. Pat. No. 3,458,530); Carbon disulfide (e.g., U.S. Pat. No. 3,256,185); Glycidol (e.g., U.S. Pat. No. 4,617,137); Urea, thiourea or guanidine (e.g., U.S. Pat. Nos. 3,312,619; 3,865,813; and British Patent GB 1,065,595); Organic sulfonic acid (e.g., U.S. Pat. No. 3,189,544 and British Patent GB 2,140,811); Alkenyl cyanide (e.g., U.S. Pat. Nos. 3,278,550 and 3,366,569); Diketene (e.g., U.S. Pat. No. 3,546,243); A diisocyanate (e.g., U.S. Pat. No. 3,573,205); Alkane sultone (e.g., U.S. Pat. No. 3,749,695); 1,3-Dicarbonyl Compound (e.g., U.S. Pat. No. 4,579,675); Sulfate of alkoxylated alcohol or phenol (e.g., U.S. Pat. No. 3,954,639); Cyclic lactone (e.g., U.S. Pat. Nos. 4,617,138; 4,645,515; 4,668,246; 4,963,275; and 4,971,711); Cyclic carbonate or thiocarbonate linear monocarbonate or polycarbonate, or chloroformate (e.g., U.S. Pat. Nos. 4,612,132; 4,647,390; 4,648,886; 4,670,170); Nitrogen-containing carboxylic acid (e.g., U.S. Pat. No. 4,971,598 and British Patent GB 2,140,811); Hydroxy-protected chlorodicarbonyloxy compound (e.g., U.S. Pat. No. 4,614,522); Lactam, thiolactam, thiolactone or dithiolactone (e.g., U.S. Pat. Nos. 4,614,603 and 4,666,460); Cyclic carbonate or thiocarbonate, linear monocarbonate or polycarbonate, or chloroformate (e.g., U.S. Pat. Nos. 4,612,132; 4,647,390; 4,646,860; and 4,670,170); Nitrogen-containing carboxylic acid (e.g., U.S. Pat. No. 4,971,598 and British Patent GB 2,440,811); Hydroxy-protected chlorodicarbonyloxy compound (e.g., U.S. Pat. No. 4,614,522); Lactam, thiolactam, thiolactone or dithiolactone (e.g., U.S. Pat. Nos. 4,614,603, and 4,666,460); Cyclic carbamate, cyclic thiocarbamate or cyclic dithiocarbamate (e.g., U.S. Pat. Nos. 4,663,062 and 4,666,459); Hydroxylaliphatic carboxylic acid (e.g., U.S. Pat. Nos. 4,482,464; 4,521,318; 4,713,189); Oxidizing agent (e.g., U.S. Pat. No. 4,379,064); Combination of phosphorus pentasulfide and a polyalkylene polyamine (e.g., U.S. Pat. No. 3,185,647); Combination of carboxylic acid or an aldehyde or ketone and sulfur or sulfur chloride (e.g., U.S. Pat. Nos. 3,390,086; 3,470,098); Combination of a hydrazine and

carbon disulfide (e.g. U.S. Pat. No. 3,519,564); Combination of an aldehyde and a phenol (e.g., U.S. Pat. Nos. 3,649,229; 5,030,249; 5,039,307); Combination of an aldehyde and an O-diester of dithiophosphoric acid (e.g., U.S. Pat. No. 3,865,740); Combination of a hydroxylaliphatic carboxylic acid and a boric acid (e.g., U.S. Pat. No. 4,554,086); Combination of a hydroxylaliphatic carboxylic acid, then formaldehyde and a phenol (e.g., U.S. Pat. No. 4,636,322); Combination of a hydroxylaliphatic carboxylic acid and then an aliphatic dicarboxylic acid (e.g., U.S. Pat. No. 4,663,064); Combination of formaldehyde and a phenol and then glycolic acid (e.g., U.S. Pat. No. 4,699,724); Combination of a hydroxylaliphatic carboxylic acid or oxalic acid and then a diisocyanate (e.g. U.S. Pat. No. 4,713,191); Combination of inorganic acid or anhydride of phosphorus or a partial or total sulfur analog thereof and a boron compound (e.g., U.S. Pat. No. 4,857,214); Combination of an organic diacid then an unsaturated fatty acid and then a nitrosoaromatic amine optionally followed by a boron compound and then a glycolating agent (e.g., U.S. Pat. No. 4,973,412); Combination of an aldehyde and a triazole (e.g., U.S. Pat. No. 4,963,278); Combination of an aldehyde and a triazole then a boron compound (e.g., U.S. Pat. No. 4,981,492); Combination of cyclic lactone and a boron compound (e.g., U.S. Pat. Nos. 4,963,275 and 4,971,711). The above-mentioned patents are herein incorporated in their entireties.

The TBN of a suitable dispersant may be from about 10 to about 65 mg KOH/g dispersant, on an oil-free basis, which is comparable to about 5 to about 30 TBN if measured on a dispersant sample containing about 50% diluent oil. TBN is measured by the method of ASTM D2896.

In yet other embodiments, the optional dispersant additive may be a hydrocarbyl substituted succinamide or succinimide dispersant. In approaches, the hydrocarbyl substituted succinamide or succinimide dispersant may be derived from a hydrocarbyl substituted acylating agent reacted with a polyalkylene polyamine and wherein the hydrocarbyl substituent of the succinamide or the succinimide dispersant is a linear or branched hydrocarbyl group having a number average molecular weight of about 250 to about 5,000 as measured by GPC using polystyrene as a calibration reference.

In some approaches, the polyalkylene polyamine used to form the dispersant has the Formula



wherein each R and R<sup>1</sup>, independently, is a divalent C1 to C6 alkylene linker, each R<sub>1</sub> and R<sub>2</sub>, independently, is hydrogen, a C1 to C6 alkyl group, or together with the nitrogen atom to which they are attached form a 5- or 6-membered ring optionally fused with one or more aromatic or non-aromatic rings, and n is an integer from 0 to 8. In other approaches, the polyalkylene polyamine is selected from the group consisting of a mixture of polyethylene polyamines having an average of 5 to 7 nitrogen atoms, triethylenetetramine, tetraethylenepentamine, and combinations thereof.

The dispersant, if present, can be used in an amount sufficient to provide up to about 20 wt %, based upon the final weight of the lubricating oil composition. Another amount of the dispersant that can be used may be about 0.1 wt % to about 15 wt %, or about 0.1 wt % to about 10 wt

%, about 0.1 to 8 wt %, or about 1 wt % to about 10 wt %, or about 1 wt % to about 8 wt %, or about 1 wt % to about 6 wt %, based upon the final weight of the lubricating oil composition. In some embodiments, the lubricating oil composition utilizes a mixed dispersant system. A single type or a mixture of two or more types of dispersants in any desired ratio may be used.

Other Antioxidants: The lubricating oil compositions herein also may optionally contain one or more antioxidants. Antioxidant compounds are known and include for example, phenates, phenate sulfides, sulfurized olefins, phosphosulfurized terpenes, sulfurized esters, aromatic amines, alkylated diphenylamines (e.g., nonyl diphenylamine, di-nonyl diphenylamine, octyl diphenylamine, di-octyl diphenylamine), phenyl-alpha-naphthylamines, alkylated phenyl-alpha-naphthylamines, hindered non-aromatic amines, phenols, hindered phenols, oil-soluble molybdenum compounds, macromolecular antioxidants, or mixtures thereof. Antioxidant compounds may be used alone or in combination.

The hindered phenol antioxidant may contain a secondary butyl and/or a tertiary butyl group as a sterically hindering group. The phenol group may be further substituted with a hydrocarbyl group and/or a bridging group linking to a second aromatic group. Examples of suitable hindered phenol antioxidants include 2,6-di-tert-butylphenol, 4-methyl-2,6-di-tert-butylphenol, 4-ethyl-2,6-di-tert-butylphenol, 4-propyl-2,6-di-tert-butylphenol or 4-butyl-2,6-di-tert-butylphenol, or 4-dodecyl-2,6-di-tert-butylphenol. In one embodiment the hindered phenol antioxidant may be an ester and may include, e.g., Irganox<sup>TM</sup> L-135 available from BASF or an addition product derived from 2,6-di-tert-butylphenol and an alkyl acrylate, wherein the alkyl group may contain about 1 to about 18, or about 2 to about 12, or about 2 to about 8, or about 2 to about 6, or about 4 carbon atoms. Another commercially available hindered phenol antioxidant may be an ester and may include Ethanol<sup>TM</sup> 4716 available from Albemarle Corporation.

Useful antioxidants may include diarylamines and high molecular weight phenols. In an embodiment, the lubricating oil composition may contain a mixture of a diarylamine and a high molecular weight phenol, such that each antioxidant may be present in an amount sufficient to provide up to about 5%, by weight, based upon the final weight of the lubricating oil composition. In an embodiment, the antioxidant may be a mixture of about 0.3 to about 1.5% diarylamine and about 0.4 to about 2.5% high molecular weight phenol, by weight, based upon the final weight of the lubricating oil composition.

Examples of suitable olefins that may be sulfurized to form a sulfurized olefin include propylene, butylene, isobutylene, polyisobutylene, pentene, hexene, heptene, octene, nonene, decene, undecene, dodecene, tridecene, tetradecene, pentadecene, hexadecene, heptadecene, octadecene, nonadecene, eicosene or mixtures thereof. In one embodiment, hexadecene, heptadecene, octadecene, nonadecene, eicosene or mixtures thereof and their dimers, trimers and tetramers are especially useful olefins. Alternatively, the olefin may be a Diels-Alder adduct of a diene such as 1,3-butadiene and an unsaturated ester, such as, butylacrylate.

Another class of sulfurized olefin includes sulfurized fatty acids and their esters. The fatty acids are often obtained from vegetable oil or animal oil and typically contain about 4 to about 22 carbon atoms. Examples of suitable fatty acids and their esters include triglycerides, oleic acid, linoleic acid, palmitoleic acid or mixtures thereof. Often, the fatty acids are obtained from lard oil, tall oil, peanut oil, soybean oil,

cottonseed oil, sunflower seed oil or mixtures thereof. Fatty acids and/or ester may be mixed with olefins, such as  $\alpha$ -olefins.

In another alternative embodiment the antioxidant composition also contains a molybdenum-containing antioxidant in addition to the phenolic and/or aminic antioxidants discussed above. When a combination of these three antioxidants is used, preferably the ratio of phenolic to aminic to molybdenum-containing component treat rates is (0 to 3):(0 to 3):(0 to 3).

The one or more antioxidant(s) may be present in ranges about 0 wt % to about 20 wt %, or about 0.1 wt % to about 10 wt %, or about 1 wt % to about 5 wt %, of the lubricating oil composition.

Other Antiwear Agents: The lubricating oil compositions herein also may optionally contain one or more antiwear agents. Examples of suitable antiwear agents include, but are not limited to, a metal thiophosphate; a metal dialkyldithiophosphate; a phosphoric acid ester or salt thereof a phosphate ester(s); a phosphite; a phosphorus-containing carboxylic ester, ether, or amide; a sulfurized olefin; thiocarbamate-containing compounds including, thiocarbamate esters, alkylene-coupled thiocarbamates, and bis(S-alkyldithiocarbamyl)disulfides; and mixtures thereof. A suitable antiwear agent may be a molybdenum dithiocarbamate. The phosphorus containing antiwear agents are more fully described in European Patent 612 839. The metal in the dialkyl dithiophosphate salts may be an alkali metal, alkaline earth metal, aluminum, lead, tin, molybdenum, manganese, nickel, copper, titanium, or zinc. A useful antiwear agent may be zinc dialkyldithiophosphate.

Further examples of suitable antiwear agents include titanium compounds, tartrates, tartrimides, oil soluble amine salts of phosphorus compounds, sulfurized olefins, phosphites (such as dibutyl phosphite), phosphonates, thiocarbamate-containing compounds, such as thiocarbamate esters, thiocarbamate amides, thiocarbamic ethers, alkylene-coupled thiocarbamates, and bis(S-alkyldithiocarbamyl)disulfides. The tartrate or tartrimide may contain alkyl-ester groups, where the sum of carbon atoms on the alkyl groups may be at least 8. The antiwear agent may in one embodiment include a citrate.

The antiwear agent may be present in ranges including about 0 wt % to about 15 wt %, or about 0.01 wt % to about 10 wt %, or about 0.05 wt % to about 5 wt %, or about 0.1 wt % to about 3 wt % of the lubricating oil composition.

Boron-Containing Compounds: The lubricating oil compositions herein may optionally contain one or more boron-containing compounds. Examples of boron-containing compounds include borate esters, borated fatty amines, borated epoxides, borated detergents, and borated dispersants, such as borated succinimide dispersants, as disclosed in U.S. Pat. No. 5,883,057. The boron-containing compound, if present, can be used in an amount sufficient to provide up to about 8 wt %, about 0.01 wt % to about 7 wt %, about 0.05 wt % to about 5 wt %, or about 0.1 wt % to about 3 wt % of the lubricating oil composition.

Other Detergents: The lubricating oil composition may optionally further comprise one or more neutral, low based, or overbased detergents, and mixtures thereof. Suitable detergent substrates include phenates, sulfur containing phenates, sulfonates, calixarates, salixarates, salicylates, carboxylic acids, phosphorus acids, mono- and/or di-thiophosphoric acids, alkyl phenols, sulfur coupled alkyl phenol compounds, or methylene bridged phenols. Suitable detergents and their methods of preparation are described in

greater detail in numerous patent publications, including U.S. Pat. No. 7,732,390 and references cited therein.

The detergent substrate may be salted with an alkali or alkaline earth metal such as, but not limited to, calcium, magnesium, potassium, sodium, lithium, barium, or mixtures thereof. In some embodiments, the detergent is free of barium. In some embodiments, a detergent may contain traces of other metals such as magnesium or calcium in amounts such as 50 ppm or less, 40 ppm or less, 30 ppm or less, 20 ppm or less, or 10 ppm or less. A suitable detergent may include alkali or alkaline earth metal salts of petroleum sulfonic acids and long chain mono- or di-alkylarylsulfonic acids with the aryl group being benzyl, tolyl, and xylyl. Examples of suitable detergents include, but are not limited to, calcium phenates, calcium sulfur containing phenates, calcium sulfonates, calcium calixarates, calcium salixarates, calcium salicylates, calcium carboxylic acids, calcium phosphorus acids, calcium mono- and/or di-thiophosphoric acids, calcium alkyl phenols, calcium sulfur coupled alkyl phenol compounds, calcium methylene bridged phenols, magnesium phenates, magnesium sulfur containing phenates, magnesium sulfonates, magnesium calixarates, magnesium salixarates, magnesium salicylates, magnesium carboxylic acids, magnesium phosphorus acids, magnesium mono- and/or di-thiophosphoric acids, magnesium alkyl phenols, magnesium sulfur coupled alkyl phenol compounds, magnesium methylene bridged phenols, sodium phenates, sodium sulfur containing phenates, sodium sulfonates, sodium calixarates, sodium salixarates, sodium salicylates, sodium carboxylic acids, sodium phosphorus acids, sodium mono- and/or di-thiophosphoric acids, sodium alkyl phenols, sodium sulfur coupled alkyl phenol compounds, or sodium methylene bridged phenols.

Overbased detergent additives are well known in the art and may be alkali or alkaline earth metal overbased detergent additives. Such detergent additives may be prepared by reacting a metal oxide or metal hydroxide with a substrate and carbon dioxide gas. The substrate is typically an acid, for example, an acid such as an aliphatic substituted sulfonic acid, an aliphatic substituted carboxylic acid, or an aliphatic substituted phenol.

The terminology "overbased" relates to metal salts, such as metal salts of sulfonates, carboxylates, and phenates, wherein the amount of metal present exceeds the stoichiometric amount. Such salts may have a conversion level in excess of 100% (i.e., they may comprise more than 100% of the theoretical amount of metal needed to convert the acid to its "normal," "neutral" salt). The expression "metal ratio," often abbreviated as MR, is used to designate the ratio of total chemical equivalents of metal in the overbased salt to chemical equivalents of the metal in a neutral salt according to known chemical reactivity and stoichiometry. In a normal or neutral salt, the metal ratio is one and in an overbased salt, MR, is greater than one. They are commonly referred to as overbased, hyperbased, or superbased salts and may be salts of organic sulfur acids, carboxylic acids, or phenols.

An overbased detergent of the lubricating oil composition may have a total base number (TBN) of about 200 mg KOH/g or greater, or as further examples, about 250 mg KOH/g or greater, or about 350 mg KOH/g or greater, or about 375 mg KOH/g or greater, or about 400 mg KOH/g or greater. The TBN being measured by the method of ASTM D2896.

Examples of suitable overbased detergents include, but are not limited to, overbased calcium phenates, overbased calcium sulfur containing phenates, overbased calcium sulfonates, overbased calcium calixarates, overbased cal-

cium salixarates, overbased calcium salicylates, overbased calcium carboxylic acids, overbased calcium phosphorus acids, overbased calcium mono- and/or di-thiophosphoric acids, overbased calcium alkyl phenols, overbased calcium sulfur coupled alkyl phenol compounds, overbased calcium methylene bridged phenols, overbased magnesium phenates, overbased magnesium sulfur containing phenates, overbased magnesium sulfonates, overbased magnesium calixarates, overbased magnesium salixarates, overbased magnesium salicylates, overbased magnesium carboxylic acids, overbased magnesium phosphorus acids, overbased magnesium mono- and/or di-thiophosphoric acids, overbased magnesium alkyl phenols, overbased magnesium sulfur coupled alkyl phenol compounds, or overbased magnesium methylene bridged phenols.

The overbased calcium phenate detergents have a total base number of at least about 150 mg KOH/g, at least about 225 mg KOH/g, at least about 225 mg KOH/g to about 400 mg KOH/g, at least about 225 mg KOH/g to about 350 mg KOH/g or about 230 mg KOH/g to about 350 mg KOH/g, all as measured by the method of ASTM D2896. When such detergent compositions are formed in an inert diluent, e.g. a process oil, usually a mineral oil, the total base number reflects the basicity of the overall composition including diluent, and any other materials (e.g., promoter, etc.) that may be contained in the detergent composition.

The overbased detergent may have a metal to substrate ratio of from 1.1:1, or from 2:1, or from 4:1, or from 5:1, or from 7:1, or from 10:1. In some embodiments, a detergent is effective at reducing or preventing rust in an engine or other automotive part such as a transmission or gear. The detergent may be present in a lubricating composition at about 0 wt % to about 10 wt %, or about 0.1 wt % to about 8 wt %, or about 1 wt % to about 4 wt %, or greater than about 4 wt % to about 8 wt %.

**Extreme Pressure Agents:** The lubricating oil compositions herein also may optionally contain one or more extreme pressure agents. Extreme Pressure (EP) agents that are soluble in the oil include sulfur- and chlorosulfur-containing EP agents, chlorinated hydrocarbon EP agents and phosphorus EP agents. Examples of such EP agents include chlorinated wax; organic sulfides and polysulfides such as dibenzyl disulfide, bis(chlorobenzyl) disulfide, dibutyl tetrasulfide, sulfurized methyl ester of oleic acid, sulfurized alkyl phenol, sulfurized dipentene, sulfurized terpene, and sulfurized Diels-Alder adducts; phosphorus-fertilized hydrocarbons such as the reaction product of phosphorus sulfide with turpentine or methyl oleate; phosphorus esters such as the dihydrocarbyl and trihydrocarbyl phosphites, e.g., dibutyl phosphite, diheptyl phosphite, dicyclohexyl phosphite, pentylphenyl phosphite; dipentylphenyl phosphite, tridecyl phosphite, distearyl phosphite and polypropylene substituted phenyl phosphite; metal thiocarbamates such as zinc dioctylthiocarbamate and barium heptylphenol diacid; amine salts of alkyl and dialkylphosphoric acids, including, for example, the amine salt of the reaction product of a dialkylthiophosphoric acid with propylene oxide; and mixtures thereof.

**Friction Modifiers:** The lubricating oil compositions herein also may optionally contain one or more friction modifiers. Suitable friction modifiers may comprise metal containing and metal-free friction modifiers and may include, but are not limited to, imidazolines, amides, amines, succinimides, alkoxylated amines, alkoxylated ether amines, amine oxides, amidoamines, nitriles, betaines, quaternary amines, imines, amine salts, amino guanadine, alkanol-amides, phosphonates, metal-containing compounds, glyc-

erol esters, sulfurized fatty compounds and olefins, sunflower oil other naturally occurring plant or animal oils, dicarboxylic acid esters, esters or partial esters of a polyol and one or more aliphatic or aromatic carboxylic acids, and the like.

Suitable friction modifiers may contain hydrocarbyl groups that are selected from straight chain, branched chain, or aromatic hydrocarbyl groups or mixtures thereof, and may be saturated or unsaturated. The hydrocarbyl groups may be composed of carbon and hydrogen or hetero atoms such as sulfur or oxygen. The hydrocarbyl groups may range from about 12 to about 25 carbon atoms. In some embodiments the friction modifier may be a long chain fatty acid ester. In another embodiment the long chain fatty acid ester may be a mono-ester, or a di-ester, or a (tri)glyceride. The friction modifier may be a long chain fatty amide, a long chain fatty ester, a long chain fatty epoxide derivatives, or a long chain imidazoline.

Other suitable friction modifiers may include organic, ashless (metal-free), nitrogen-free organic friction modifiers. Such friction modifiers may include esters formed by reacting carboxylic acids and anhydrides with alkanols and generally include a polar terminal group (e.g. carboxyl or hydroxyl) covalently bonded to an oleophilic hydrocarbon chain. An example of an organic ashless nitrogen-free friction modifier is known generally as glycerol monooleate (GMO) which may contain mono-, di-, and tri-esters of oleic acid. Other suitable friction modifiers are described in U.S. Pat. No. 6,723,685, herein incorporated by reference in its entirety.

Aminic friction modifiers may include amines or polyamines. Such compounds can have hydrocarbyl groups that are linear, either saturated or unsaturated, or a mixture thereof and may contain from about 12 to about 25 carbon atoms. Further examples of suitable friction modifiers include alkoxylated amines and alkoxylated ether amines. Such compounds may have hydrocarbyl groups that are linear, either saturated, unsaturated, or a mixture thereof. They may contain from about 12 to about 25 carbon atoms. Examples include ethoxylated amines and ethoxylated ether amines.

The amines and amides may be used as such or in the form of an adduct or reaction product with a boron compound such as a boric oxide, boron halide, metaborate, boric acid or a mono-, di- or tri-alkyl borate. Other suitable friction modifiers are described in U.S. Pat. No. 6,300,291, herein incorporated by reference in its entirety.

A friction modifier may optionally be present in ranges such as about 0 wt % to about 10 wt %, or about 0.01 wt % to about 8 wt %, or about 0.1 wt % to about 4 wt %.

**Molybdenum-containing component:** The lubricating oil compositions herein also may optionally contain one or more molybdenum-containing compounds. An oil-soluble molybdenum compound may have the functional performance of an antiwear agent, an antioxidant, a friction modifier, or mixtures thereof. An oil-soluble molybdenum compound may include molybdenum dithiocarbamates, molybdenum dialkyldithiophosphates, molybdenum dithiophosphinates, amine salts of molybdenum compounds, molybdenum xanthates, molybdenum thioxanthates, molybdenum sulfides, molybdenum carboxylates, molybdenum alkoxides, a trinuclear organo-molybdenum compound, and/or mixtures thereof. The molybdenum sulfides include molybdenum disulfide. The molybdenum disulfide may be in the form of a stable dispersion. In one embodiment the oil-soluble molybdenum compound may be selected from the group consisting of molybdenum dithiocarbamates,

molybdenum dialkyldithiophosphates, amine salts of molybdenum compounds, and mixtures thereof. In one embodiment the oil-soluble molybdenum compound may be a molybdenum dithiocarbamate.

5 Suitable examples of molybdenum compounds which may be used include commercial materials sold under the trade names such as Molyvan® 822, Molyvan® A, Molyvan® 2000, Molyvan® 855, Molyvan® 1055, and Molyvan® 3000 from R. T. Vanderbilt Co., Ltd., and Adeka 10 10 Sakura-Lube® S-165, S-200, S-300, S-310G, S-525, S-600, S-700, and S-710 available from Adeka Corporation, and mixtures thereof. Suitable molybdenum components are described in U.S. Pat. No. 5,650,381; US RE 37,363 E1; US RE 38,929 E1; and US RE 40,595 E1, incorporated herein 15 by reference in their entireties.

Additionally, the molybdenum compound may be an acidic molybdenum compound. Included are molybdic acid, ammonium molybdate, sodium molybdate, potassium molybdate, and other alkaline metal molybdates and other 20 molybdenum salts, e.g., hydrogen sodium molybdate,  $\text{MoOCl}_4$ ,  $\text{MoO}_2\text{Br}_2$ ,  $\text{Mo}_2\text{O}_3\text{Cl}_6$ , molybdenum trioxide or similar acidic molybdenum compounds. Alternatively, the compositions can be provided with molybdenum by molybdenum/sulfur complexes of basic nitrogen compounds as 25 described, for example, in U.S. Pat. Nos. 4,263,152; 4,285, 822; 4,283,295; 4,272,387; 4,265,773; 4,261,843; 4,259,195 and 4,259,194; and WO 94/06897, incorporated herein by reference in their entireties.

Another class of suitable organo-molybdenum compounds are trinuclear molybdenum compounds, such as 30 those of the formula  $\text{Mo}_3\text{S}_k\text{L}_n\text{Q}_z$  and mixtures thereof, wherein S represents sulfur, L represents independently selected ligands having organo groups with a sufficient number of carbon atoms to render the compound soluble or 35 dispersible in the oil, n is from 1 to 4, k varies from 4 through 7, Q is selected from the group of neutral electron donating compounds such as water, amines, alcohols, phosphines, and ethers, and z ranges from 0 to 5 and includes non-stoichiometric values. At least 21 total carbon atoms 40 may be present among all the ligands' organo groups, such as at least 25, at least 30, or at least 35 carbon atoms. Additional suitable molybdenum compounds are described in U.S. Pat. No. 6,723,685, herein incorporated by reference in its entirety.

45 The oil-soluble molybdenum compound may be present in an amount sufficient to provide about 0.5 ppm to about 2000 ppm, about 1 ppm to about 700 ppm, about 1 ppm to about 550 ppm, about 5 ppm to about 300 ppm, or about 20 ppm to about 250 ppm of molybdenum.

50 **Transition Metal-containing compounds:** In another embodiment, the oil-soluble compound may be a transition metal containing compound or a metalloid. The transition metals may include, but are not limited to, titanium, vanadium, copper, zinc, zirconium, molybdenum, tantalum, tungsten, and the like. Suitable metalloids include, but are 55 not limited to, boron, silicon, antimony, tellurium, and the like.

50 In an embodiment, an oil-soluble transition metal-containing compound may function as antiwear agents, friction 60 modifiers, antioxidants, deposit control additives, or more than one of these functions. In an embodiment the oil-soluble transition metal-containing compound may be an oil-soluble titanium compound, such as a titanium (IV) alkoxide. Among the titanium containing compounds that 65 may be used in, or which may be used for preparation of the oil-soluble materials of, the disclosed technology are various Ti (IV) compounds such as titanium (IV) oxide; titanium

(IV) sulfide; titanium (IV) nitrate; titanium (IV) alkoxides such as titanium methoxide, titanium ethoxide, titanium propoxide, titanium isopropoxide, titanium butoxide, titanium 2-ethylhexoxide; and other titanium compounds or complexes including but not limited to titanium phenates; titanium carboxylates such as titanium (IV) 2-ethyl-1-3-hexanedioate or titanium citrate or titanium oleate; and titanium (IV) (triethanolaminato)isopropoxide. Other forms of titanium encompassed within the disclosed technology include titanium phosphates such as titanium dithiophosphates (e.g., dialkyldithiophosphates) and titanium sulfonates (e.g., alkylbenzenesulfonates), or, generally, the reaction product of titanium compounds with various acid materials to form salts, such as oil-soluble salts. Titanium compounds can thus be derived from, among others, organic acids, alcohols, and glycols. Ti compounds may also exist in dimeric or oligomeric form, containing Ti—O—Ti structures. Such titanium materials are commercially available or can be readily prepared by appropriate synthesis techniques which will be apparent to the person skilled in the art. They may exist at room temperature as a solid or a liquid, depending on the particular compound. They may also be provided in a solution form in an appropriate inert solvent.

In one embodiment, the titanium can be supplied as a Ti-modified dispersant, such as a succinimide dispersant. Such materials may be prepared by forming a titanium mixed anhydride between a titanium alkoxide and a hydrocarbyl-substituted succinic anhydride, such as an alkenyl-(or alkyl) succinic anhydride. The resulting titanate-succinate intermediate may be used directly or it may be reacted with any of a number of materials, such as (a) a polyamine-based succinimide/amide dispersant having free, condensable —NH functionality; (b) the components of a polyamine-based succinimide/amide dispersant, i.e., an alkenyl-(or alkyl) succinic anhydride and a polyamine, (c) a hydroxy-containing polyester dispersant prepared by the reaction of a substituted succinic anhydride with a polyol, aminoalcohol, polyamine, or mixtures thereof. Alternatively, the titanate-succinate intermediate may be reacted with other agents such as alcohols, aminoalcohols, ether alcohols, polyether alcohols or polyols, or fatty acids, and the product thereof either used directly to impart Ti to a lubricant, or else further reacted with the succinic dispersants as described above. As an example, 1 part (by mole) of tetraisopropyl titanate may be reacted with about 2 parts (by mole) of a polyisobutene-substituted succinic anhydride at 140-150° C. for 5 to 6 hours to provide a titanium modified dispersant or intermediate. The resulting material (30 g) may be further reacted with a succinimide dispersant from polyisobutene-substituted succinic anhydride and a polyethylenepolyamine mixture (127 grams+diluent oil) at 150° C. for 1.5 hours, to produce a titanium-modified succinimide dispersant.

Another titanium containing compound may be a reaction product of titanium alkoxide and C<sub>6</sub> to C<sub>25</sub> carboxylic acid. The reaction product may be represented by the following formula:



wherein n is an integer selected from 2, 3 and 4, and R is a hydrocarbyl group containing from about 5 to about 24 carbon atoms, or by the formula:



wherein m+n=4 and n ranges from 1 to 3, R<sub>4</sub> is an alkyl moiety with carbon atoms ranging from 1-8, R<sub>1</sub> is selected from a hydrocarbyl group containing from about 6 to 25 carbon atoms, and R<sub>2</sub> and R<sub>3</sub> are the same or different and are selected from a hydrocarbyl group containing from about 1 to 6 carbon atoms, or the titanium compound may be represented by the formula:



wherein x ranges from 0 to 3, R<sub>1</sub> is selected from a hydrocarbyl group containing from about 6 to 25 carbon atoms, R<sub>2</sub>, and R<sub>3</sub> are the same or different and are selected from a hydrocarbyl group containing from about 1 to 6 carbon atoms, and R<sub>4</sub> is selected from a group consisting of either H, or C<sub>6</sub> to C<sub>25</sub> carboxylic acid moiety.

Suitable carboxylic acids may include, but are not limited to caproic acid, caprylic acid, lauric acid, myristic acid, palmitic acid, stearic acid, arachidic acid, oleic acid, erucic acid, linoleic acid, linolenic acid, cyclohexanecarboxylic acid, phenylacetic acid, benzoic acid, neodecanoic acid, and the like.

In an embodiment the oil soluble titanium compound may be present in the lubricating oil composition in an amount to provide from 0 to 3000 ppm titanium by weight or 25 to about 1500 ppm titanium by weight or about 35 ppm to 500 ppm titanium by weight or about 50 ppm to about 300 ppm.

**Viscosity Index Improvers:** The lubricating oil compositions herein also may optionally contain one or more viscosity index improvers. Suitable viscosity index improvers may include polyolefins, olefin copolymers, ethylene/propylene copolymers, polyisobutenes, hydrogenated styrene-isoprene polymers, styrene/maleic ester copolymers, hydrogenated styrene/butadiene copolymers, hydrogenated isoprene polymers, alpha-olefin maleic anhydride copolymers, polymethacrylates, polyacrylates, polyalkyl styrenes, hydrogenated alkenyl aryl conjugated diene copolymers, or mixtures thereof. Viscosity index improvers may include star polymers and suitable examples are described in US Publication No. 20120101017A1.

The lubricating oil compositions herein also may optionally contain one or more dispersant viscosity index improvers in addition to a viscosity index improver or in lieu of a viscosity index improver. Suitable viscosity index improvers may include functionalized polyolefins, for example, ethyl-

ene-propylene copolymers that have been functionalized with the reaction product of an acylating agent (such as maleic anhydride) and an amine; polymethacrylates functionalized with an amine, or esterified maleic anhydride-styrene copolymers reacted with an amine.

The total amount of viscosity index improver and/or dispersant viscosity index improver may be about 0 wt % to about 20 wt %, about 0.1 wt % to about 15 wt %, about 0.1 wt % to about 12 wt %, or about 0.5 wt % to about 10 wt %, of the lubricating oil composition.

Other Optional Additives: Other additives may be selected to perform one or more functions required of a lubricating fluid. Further, one or more of the mentioned additives may be multi-functional and provide functions in addition to or other than the function prescribed herein.

A lubricating oil composition according to the present disclosure may optionally comprise other performance additives. The other performance additives may be in addition to specified additives of the present disclosure and/or may comprise one or more of metal deactivators, viscosity index improvers, detergents, ashless TBN boosters, friction modifiers, antiwear agents, corrosion inhibitors, rust inhibitors, dispersants, dispersant viscosity index improvers, extreme pressure agents, antioxidants, foam inhibitors, demulsifiers, emulsifiers, pour point depressants, seal swelling agents and mixtures thereof. Typically, fully-formulated lubricating oil will contain one or more of these performance additives.

Suitable metal deactivators may include derivatives of benzotriazoles (typically tolyltriazole), dimercaptothiadiazole derivatives, 1,2,4-triazoles, benzimidazoles, 2-alkyldithiobenzimidazoles, or 2-alkyldithiobenzothiazoles; foam inhibitors including copolymers of ethyl acrylate and 2-ethylhexylacrylate and optionally vinyl acetate; demulsifiers including trialkyl phosphates, polyethylene glycols, polyethylene oxides, polypropylene oxides and (ethylene oxide-propylene oxide) polymers; pour point depressants including esters of maleic anhydride-styrene, polymethacrylates, polyacrylates or polyacrylamides.

Suitable foam inhibitors include silicon-based compounds, such as siloxane.

Suitable pour point depressants may include polymethylmethacrylates or mixtures thereof. Pour point depressants may be present in an amount sufficient to provide from about 0 wt % to about 1 wt %, about 0.01 wt % to about 0.5 wt %, or about 0.02 wt % to about 0.04 wt % based upon the final weight of the lubricating oil composition.

Suitable rust inhibitors may be a single compound or a mixture of compounds having the property of inhibiting corrosion of ferrous metal surfaces. Non-limiting examples of rust inhibitors useful herein include oil-soluble high molecular weight organic acids, such as 2-ethylhexanoic acid, lauric acid, myristic acid, palmitic acid, oleic acid, linoleic acid, linolenic acid, behenic acid, and cerotic acid, as well as oil-soluble polycarboxylic acids including dimer and trimer acids, such as those produced from tall oil fatty acids, oleic acid, and linoleic acid. Other suitable corrosion inhibitors include long-chain alpha, omega-dicarboxylic acids in the molecular weight range of about 600 to about 3000 and alkenylsuccinic acids in which the alkenyl group contains about 10 or more carbon atoms such as, tetrapropenylsuccinic acid, tetradecenylsuccinic acid, and hexadecenylsuccinic acid. Another useful type of acidic corrosion inhibitors are the half esters of alkenyl succinic acids having about 8 to about 24 carbon atoms in the alkenyl group with alcohols such as the polyglycols. The corresponding half amides of such alkenyl succinic acids are also useful. A useful rust inhibitor is a high molecular weight organic acid.

The rust inhibitor, if present, can be used in an amount sufficient to provide about 0 wt % to about 5 wt %, about 0.01 wt % to about 3 wt %, about 0.1 wt % to about 2 wt %, based upon the final weight of the lubricating oil composition.

In general terms, a suitable lubricant including the detergent metals herein may include additive components in the ranges listed in the following table.

10

TABLE 2

| Suitable Lubricating Compositions          |                                 |                                 |
|--------------------------------------------|---------------------------------|---------------------------------|
| Component                                  | Wt. %<br>(Suitable Embodiments) | Wt. %<br>(Suitable Embodiments) |
| Detergent Systems                          | 0.02-5.0                        | 0.2-2.0                         |
| Dispersant Systems                         | 0-8.0                           | 1-6.0                           |
| Antioxidant(s)                             | 0.1-5.0                         | 0.01-3.0                        |
| Ashless TBN booster(s)                     | 0.0-1.0                         | 0.01-0.5                        |
| Corrosion inhibitor(s)                     | 0.0-5.0                         | 0.0-2.0                         |
| 20 Metal dihydrocarbyl-dithiophosphates(s) | 0.0-6.0                         | 0.1-4.0                         |
| Ash-free phosphorus compound(s)            | 0.0-6.0                         | 0.0-4.0                         |
| Antifoaming agent(s)                       | 0.0-5.0                         | 0.001-0.15                      |
| Antiwear agent(s)                          | 0.0-1.0                         | 0.0-0.8                         |
| 25 Pour point depressant(s)                | 0.0-5.0                         | 0.01-1.5                        |
| Viscosity index improver(s)                | 0.0-25.0                        | 0.1-15.0                        |
| Dispersant viscosity index improver(s)     | 0.0-10.0                        | 0.0-5.0                         |
| Friction modifier(s)                       | 0.00-5.0                        | 0.01-2.0                        |
| 30 Base oil                                | Balance                         | Balance                         |
| Total                                      | 100                             | 100                             |

30

The percentages of each component above represent the weight percent of each component, based upon the weight of the final lubricating oil composition. The remainder of the lubricating oil composition consists of one or more base oils. Additives used in formulating the compositions described herein may be blended into the base oil individually or in various sub-combinations. However, it may be suitable to blend all of the components concurrently using an additive concentrate (i.e., additives plus a diluent, such as a hydrocarbon solvent). Fully formulated lubricants conventionally contain an additive package, referred to herein as a dispersant/inhibitor package or DI package, that will supply the characteristics that are required in the formulation.

45

### Definitions

For purposes of this disclosure, the chemical elements are identified in accordance with the Periodic Table of the Elements, CAS version, Handbook of Chemistry and Physics, 75th Ed. Additionally, general principles of organic chemistry are described in "Organic Chemistry", Thomas Sorrell, University Science Books, Sausalito: 1999, and 50 "March's Advanced Organic Chemistry", 5th Ed., Ed.: Smith, M. B. and March, J., John Wiley & Sons, New York: 2001, the entire contents of which are hereby incorporated by reference.

As described herein, compounds may optionally be substituted with one or more substituents, such as are illustrated generally above, or as exemplified by particular classes, subclasses, and species of the disclosure.

Unless otherwise apparent from the context, the term "major amount" is understood to mean an amount greater than or equal to 50 weight percent, for example, from about 60 80 to about 98 weight percent relative to the total weight of the composition. Moreover, as used herein, the term "minor

amount" is understood to mean an amount less than 50 weight percent relative to the total weight of the composition.

As used herein, the term "hydrocarbyl group" or "hydrocarbyl" is used in its ordinary sense, which is well-known to those skilled in the art. Specifically, it refers to a group having a carbon atom directly attached to the remainder of a molecule and having a predominantly hydrocarbon character. Examples of hydrocarbyl groups include: (1) hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form an alicyclic radical); (2) substituted hydrocarbon substituents, that is, substituents containing non-hydrocarbon groups which, in the context of the description herein, do not alter the predominantly hydrocarbon substituent (e.g., halo (especially chloro and fluoro), hydroxy, alkoxy, mercapto, alkylmercapto, nitro, nitroso, amino, alkylamino, and sulfoxyl); (3) hetero-substituents, that is, substituents which, while having a predominantly hydrocarbon character, in the context of this description, contain other than carbon in a ring or chain otherwise composed of carbon atoms. Hetero-atoms include sulfur, oxygen, nitrogen, and encompass substituents such as pyridyl, furyl, thienyl, and imidazolyl. In general, no more than two, or as a further example, no more than one, non-hydrocarbon substituent will be present for every ten carbon atoms in the hydrocarbyl group; in some embodiments, there will be no non-hydrocarbon substituent in the hydrocarbyl group.

As used herein the term "aliphatic" encompasses the terms alkyl, alkenyl, alkynyl, each of which being optionally substituted as set forth below.

As used herein, an "alkyl" group refers to a saturated aliphatic hydrocarbon group containing 1-12 (e.g., 1-8, 1-6, or 1-4) carbon atoms. An alkyl group can be straight or branched. Examples of alkyl groups include, but are not limited to, methyl, ethyl, propyl, isopropyl, butyl, isobutyl, sec-butyl, tert-butyl, n-pentyl, n-heptyl, or 2-ethylhexyl. An alkyl group can be substituted (i.e., optionally substituted) with one or more substituents such as halo, phospho, cycloaliphatic [e.g., cycloalkyl or cycloalkenyl], heterocycloaliphatic [e.g., heterocycloalkyl or heterocycloalkenyl], aryl, heteroaryl, alkoxy, aryl, heteroaryl, acyl [e.g., (aliphatic) carbonyl, (cycloaliphatic)carbonyl, or (heterocycloaliphatic) carbonyl], nitro, cyano, amido [e.g., (cycloalkylalkyl)carbonylamino, arylcarbonylamino, aralkylcarbonylamino, (heterocycloalkyl) carbonylamino, (heterocycloalkylalkyl) carbonylamino, heteroarylcarbonylamino, heteroaralkylcarbonylamino, heteroalkylaminocarbonyl, arylaminocarbonyl, or heteroarylamino], sulfonyl [e.g., aliphatic-SO<sub>2</sub>—], sulfinyl, sulfanyl, sulfoxyl, urea, thiourea, sulfamoyl, sulfamide, oxo, carboxy, carbamoyl, cycloaliphaticoxy, heterocycloaliphaticoxy, aryloxy, heteroaryloxy, aralkyloxy, heteroaralkoxy, alkoxy carbonyl, alkylcarbonyloxy, or hydroxy. Without limitation, some examples of substituted alkyls include carboxyalkyl (such as HOOC-alkyl, alkoxy carbonylalkyl, and alkylcarbonyloxy-alkyl), cyanoalkyl, hydroxyalkyl, alkoxyalkyl, acylalkyl, aralkyl, (alkoxyaryl)alkyl, (sulfonylamino) alkyl (such as (alkyl-SO<sub>2</sub>-amino)alkyl), aminoalkyl, amidoalkyl, (cycloaliphatic)alkyl, or haloalkyl.

As used herein, an "alkenyl" group refers to an aliphatic carbon group that contains 2-8 (e.g., 2-12, 2-6, or 2-4) carbon atoms and at least one double bond. Like an alkyl group, an alkenyl group can be straight or branched. Examples of an alkenyl group include, but are not limited to allyl, isoprenyl, 2-butenyl, and 2-hexenyl. An alkenyl group can be optionally substituted with one or more substituents such as halo, phospho, cycloaliphatic [e.g., cycloalkyl or cycloalkenyl], heterocycloaliphatic [e.g., heterocycloalkyl or heterocycloalkenyl], aryl, heteroaryl, alkoxy, aryl, heteroaryl, acyl [e.g., (aliphatic) carbonyl, (cycloaliphatic) carbonyl, or (heterocycloaliphatic) carbonyl], nitro, cyano, amido [e.g., (cycloalkylalkyl)carbonylamino, arylcarbonylamino, aralkylcarbonylamino, (heterocycloalkylalkyl) carbonylamino, heteroaralkylcarbonylamino, heteroarylcarbonylamino, heteroaralkylcarbonylamino, alkylamino carbonyl, cycloalkylaminocarbonyl, hetero cyclo alkylaminocarbonyl, arylaminocarbonyl, or heteroarylamino carbonyl], amino [e.g., aliphaticamino, cycloaliphaticamino, heterocyclo aliphaticamino, or aliphaticsulfonylamino], sulfonyl [e.g., alkyl-SO<sub>2</sub>—, cycloaliphatic-SO<sub>2</sub>—, or aryl-SO<sub>2</sub>—], sulfinyl, sulfanyl, sulfoxyl, urea, thiourea, sulfamoyl, sulfamide, oxo, carboxy, carbamoyl, cycloaliphaticoxy, heterocycloaliphaticoxy, aryloxy, heteroaryloxy, aralkyloxy, heteroaralkoxy, alkoxy carbonyl, alkylcarbonyloxy, or hydroxy. Without limitation, some examples of substituted alkenyls include cyanoalkenyl, alkoxyalkenyl, acylalkenyl, hydroxyl alkenyl, aralkenyl, (alkoxyaryl) alkenyl, (sulfonylamino)alkenyl (such as (alkyl-SO<sub>2</sub>-amino) alkenyl), aminoalkenyl, amidoalkenyl, (cycloaliphatic)alkenyl, or haloalkenyl.

As used herein, an "alkynyl" group refers to an aliphatic carbon group that contains 2-8 (e.g., 2-12, 2-6, or 2-4) carbon atoms and has at least one triple bond. An alkynyl group can be straight or branched. Examples of an alkynyl group include, but are not limited to, propargyl and butynyl. An alkynyl group can be optionally substituted with one or more substituents such as aryl, heteroaryl, alkoxy, cycloalkyloxy, heterocycloalkyloxy, aryloxy, heteroaryloxy, aralkyloxy, nitro, carboxy, cyano, halo, hydroxy, sulfo, mercapto, sulfanyl [e.g., aliphatic sulfanyl or cycloaliphatic sulfanyl], sulfinyl [e.g., aliphatic sulfinyl or cycloaliphatic sulfinyl], sulfonyl [e.g., aliphatic-SO<sub>2</sub>—, aliphaticamino-SO<sub>2</sub>—, or cycloaliphatic-SO<sub>2</sub>—], amido [e.g., aminocarbonyl, alkylaminocarbonyl, alkylcarbonylamino, cyclo alkylaminocarbonyl, heterocycloalkylaminocarbonyl, cycloalkylcarbonylamino, arylamino carbonyl, arylcarbonylamino, aralkylcarbonylamino, (heterocycloalkyl) carbonylamino, heteroaralkylcarbonylamino, heteroaryl carbonylamino or heteroaryl amino carbonyl], urea, thiourea, sulfamoyl, sulfamide, alkoxy carbonyl, alkyl carbonyloxy, cyclo aliphatic, heterocycloaliphatic, aryl, heteroaryl, acyl [e.g., (cycloaliphatic) carbonyl or (heterocycloaliphatic) carbonyl], amino [e.g., aliphaticamino], sulfoxyl, oxo, carboxy, carbamoyl, (cycloaliphatic)oxy, (heterocycloaliphatic)oxy, or (heteroaryl) alkoxy.

As used herein, an "amino" group refers to —NR<sup>X</sup>R<sup>Y</sup> wherein each of R<sup>X</sup> and R<sup>Y</sup> is independently hydrogen, alkyl, cycloalkyl, (cycloalkyl)alkyl, aryl, aralkyl, heterocycloalkyl, (heterocycloalkyl)alkyl, heteroaryl, carboxy, sulfanyl, sulfinyl, sulfonyl, (alkyl)carbonyl, (cycloalkyl)carbonyl, ((cycloalkyl)alkyl)carbonyl, arylcarbonyl, (aralkyl)carbonyl, (heterocycloalkyl)carbonyl, ((heterocycloalkyl)alkyl)carbonyl, (heteroaryl)carbonyl, or (heteroaralkyl) carbonyl, each of which being defined herein and being optionally substituted. Examples of amino groups include alkylamino,

dialkylamino, or arylamino. When the term "amino" is not the terminal group (e.g., alkylcarbonylamino), it is represented by  $-\text{NR}^X-$ .  $\text{R}^X$  has the same meaning as defined above.

As used herein, a "cycloalkyl" group refers to a saturated carbocyclic mono- or bicyclic (fused or bridged) ring of 3-10 (e.g., 5-10) carbon atoms. Examples of cycloalkyl groups include cyclopropyl, cyclobutyl, cyclopentyl, cyclohexyl, cycloheptyl, adamantyl, norbornyl, cubyl, octahydroindenyl, decahydro-naphthyl, bicyclo[3.2.1]octyl, bicyclo [2.2.2] octyl, bicyclo[3.3.1]nonyl, bicyclo[3.3.2.] decyl, bicyclo[2.2.2]octyl, adamantyl, or ((aminocarbonyl)cycloalkyl)cycloalkyl.

As used herein, a "heterocycloalkyl" group refers to a 3-10 membered mono- or bicyclic (fused or bridged) (e.g., 5- to 10-membered mono- or bicyclic) saturated ring structure, in which one or more of the ring atoms is a heteroatom (e.g., N, O, S, or combinations thereof). Examples of a heterocycloalkyl group include piperidyl, piperazyl, tetrahydropyranyl, tetrahydrofuryl, 1,4-dioxolanyl, 1,4-dithianyl, 1,3-dioxolanyl, oxazolidyl, isoxazolidyl, morpholinyl, thiomorpholyl, octahydrobenzofuryl, octahydrochromenyl, octahydrothio chromenyl, octahydroindolyl, octahydpyrindinyl, decahydroquinolinolyl, octahydrobenzo[b] thio-phenetyl, 2-oxa-bicyclo[2.2.2]octyl, 1-aza-bicyclo[2.2.2]octyl, 3-aza-bicyclo[3.2.1]octyl, and 2,6-dioxa-tricyclo [3.3.1.0]nonyl. A monocyclic heterocycloalkyl group can be fused with a phenyl moiety to form structures, such as tetrahydroisoquinoline, which would be categorized as heteroaryls.

A "heteroaryl" group, as used herein, refers to a monocyclic, bicyclic, or tricyclic ring system having 4 to 15 ring atoms wherein one or more of the ring atoms is a heteroatom (e.g., N, O, S, or combinations thereof) and in which the monocyclic ring system is aromatic or at least one of the rings in the bicyclic or tricyclic ring systems is aromatic. A heteroaryl group includes a benzofused ring system having 2 to 3 rings. For example, a benzofused group includes benzo fused with one or two 4 to 8 membered heterocycloaliphatic moieties (e.g., indolizyl, indolyl, isoindolyl, 3H-indolyl, indolinyl, benzo[b]furyl, benzo[b]thiophenyl, quinolinyl, or isoquinolinyl). Some examples of heteroaryl are pyridyl, 1H-indazolyl, furyl, pyrrolyl, thieryl, thiazolyl, oxazolyl, imidazolyl, tetrazolyl, benzofuryl, isoquinolinyl, benzthiazolyl, xanthene, thioxanthene, phenothiazine, dihydroindole, benzo[1,3]dioxole, benzo[b]furyl, benzo[b] thiophenyl, indazolyl, benzimidazolyl, benzthiazolyl, puryl, cinnolyl, quinolyl, quinazolyl, cinnolyl, phthalazyl, quinazolyl, quinoxalyl, isoquinolyl, 4H-quinolizyl, benzo-1,2,5-thiadiazolyl, or 1,8-naphthyridyl.

Without limitation, monocyclic heteroaryls include furyl, thiophenyl, 2H-pyrrolyl, pyrrolyl, oxazolyl, thiazolyl, imidazolyl, pyrazolyl, isoxazolyl, isothiazolyl, 1,3,4-thiadiazolyl, 2H-pyranyl, 4-H-pranyl, pyridyl, pyridazyl, pyrimidyl, pyrazolyl, pyrazyl, or 1,3,5-triazyl. Monocyclic heteroaryls are numbered according to standard chemical nomenclature.

Without limitation, bicyclic heteroaryls include indolizyl, indolyl, isoindolyl, 3H-indolyl, indolinyl, benzo[b]furyl, benzo[b]thiophenyl, quinolinyl, isoquinolinyl, indolizinyl, isoindolyl, indolyl, benzo[b]furyl, bexo[b]thiophenyl, indazolyl, benzimidazolyl, benzthiazolyl, purinyl, 4H-quinolizyl, quinolyl, isoquinolyl, cinnolyl, phthalazyl, quinazolyl, quinoxalyl, 1,8-naphthyridyl, or pteridyl. Bicyclic heteroaryls are numbered according to standard chemical nomenclature.

As used herein, the term "treat rate" refers to the weight percent of a component in the finished lubricant or the passenger car motor oil.

The weight average molecular weight (Mw) and the number average molecular weight (Mn) may be determined with a gel permeation chromatography (GPC) instrument obtained from Waters or the like instrument and the data processed with Waters Empower Software or the like software. The GPC instrument may be equipped with a Waters Separations Module and Waters Refractive Index detector (or the like optional equipment). The GPC operating conditions may include a guard column, 4 Agilent PLgel columns (length of 300 $\times$ 7.5 mm; particle size of 5  $\mu$ m, and pore size ranging from 100-1000  $\text{\AA}$ ) with the column temperature at about 40° C. Un-stabilized HPLC grade tetrahydrofuran (THF) may be used as solvent, at a flow rate of 1.0 mL/min. The GPC instrument may be calibrated with commercially available poly(methyl methacrylate) (PMMA) standards having a narrow molecular weight distribution ranging from 960-1,568,000 g/mol. The calibration curve can be extrapolated for samples having a mass less than 500 g/mol. Samples and PMMA standards can be in dissolved in THF and prepared at concentration of 0.1 to 0.5 wt. % and used without filtration. GPC measurements are also described in U.S. Pat. No. 5,266,223, which is incorporated herein by reference. The GPC method additionally provides molecular weight distribution information; see, for example, W. W. Yau, J. J. Kirkland and D. D. Bly, "Modern Size Exclusion Liquid Chromatography", John Wiley and Sons, New York, 1979, also incorporated herein by reference.

## EXAMPLES

A better understanding of the present disclosure and its many advantages may be clarified with the following examples. The following examples are illustrative and not limiting thereof in either scope or spirit. Those skilled in the art will readily understand that variations of the components, methods, steps, and devices described in these examples can be used. Unless noted otherwise or apparent from the context of discussion in the Examples below and throughout this disclosure, all percentages, ratios, and parts noted in this disclosure are by weight. KV100 is measured herein pursuant to ASTM D445.

### Example 1

Inventive and Comparative additive packages for lubricants were prepared including the following dispersant, detergent, ZDDPs, and viscosity index improvers:

Polysisobutylene succinimide dispersant A derived from a highly reactive polysisobutylene having a number average molecular weight of about 2000 to about 2600 and having about 1.5 weight percent nitrogen.

Polysisobutylene succinimide dispersant B derived from a highly reactive polysisobutylene having a number average molecular weight of about 1200 to about 1800 and having about 1.6 weight percent nitrogen and posted treated with maleic anhydride and a boron source so that the dispersant has about 0.8 weight percent boron.

Overbased Magnesium sulfonate detergent having a TBN of 400 and having a soap content of about 29 percent.

Overbased calcium sulfonate detergent having a TBN of 300 and a soap content of about 26 percent.

ZDDP A was a zinc dialkyldithiophosphate and included alkyl groups derived from a secondary alcohol.

ZDDP B was a zinc dialkyldithiophosphate and included alkyl groups derived from a primary alcohol.

In addition to the above components, the Comparative and Inventive additive packages of this Example also

included other common additives suitable for passenger car motor oils and were the same for each evaluated additive package. The only variations in the additive packages of this Example were the above noted components to derive the fluid relationships of Table 3 below.

TABLE 3

| Fluid Relationships of Additive Packages |             |             |             |       |
|------------------------------------------|-------------|-------------|-------------|-------|
|                                          | Comparative | Inventive 1 | Inventive 2 |       |
| <b>Overall Calculations</b>              |             |             |             |       |
| Boron (B)                                | % Wt.       | 0.023       | 0.014       | 0.014 |
| Calcium                                  | % Wt.       | 0.131       | 0.101       | 0.102 |
| Magnesium                                | % Wt.       | 0.058       | 0.056       | 0.057 |
| Nitrogen                                 | % Wt.       | 0.099       | 0.111       | 0.111 |
| Phosphorus                               | % Wt.       | 0.077       | 0.075       | 0.065 |
| Zinc                                     | % Wt.       | 0.085       | 0.082       | 0.072 |
| Sulphated Ash                            | % Wt.       | 0.924       | 0.775       | 0.781 |
| TBN                                      | mg KOH/g    | 8.18        | 8.00        | 7.97  |
| Ca:Mg                                    |             | 2.26        | 1.79        | 1.78  |
| Dispersant calculations                  |             |             |             |       |
| Nitrogen (N)                             | % Wt.       | 0.068       | 0.061       | 0.063 |
| Boron (B)                                | % Wt.       | 0.023       | 0.014       | 0.014 |
| TBN                                      | mg KOH/g    | 1.323       | 1.166       | 1.194 |
| Disp B/(Disp TBN*Disp N)                 |             | 0.259       | 0.191       | 0.192 |
| Detergent calculations                   |             |             |             |       |
| Calcium Soap                             | % Wt.       | 0.286       | 0.221       | 0.224 |
| Magnesium Soap                           | % Wt.       | 0.172       | 0.168       | 0.171 |
| Sulphonate soap                          | % Wt.       | 0.458       | 0.389       | 0.395 |
| Phenate soap                             | % Wt.       | 0           | 0           | 0     |
| Total Soap                               | % Wt.       | 0.458       | 0.389       | 0.395 |
| TBN                                      | mg KOH/g    | 5.804       | 4.987       | 5.059 |
| Ca:Mg Soap                               |             | 1.666       | 1.314       | 1.307 |
| Elemental Ca:Total Soap                  |             | 0.286       | 0.259       | 0.259 |
| Ca Soap: Total Soap                      |             | 0.624       | 0.568       | 0.566 |
| ZDDP calculations                        |             |             |             |       |
| Primary ZDDP                             | %           | 20.53       | 36.03       | 36.08 |
| Secondary ZDDP                           | %           | 79.47       | 63.96       | 63.92 |
| Prim:Sec                                 |             | 0.26        | 0.56        | 0.56  |
| Ave Carbon:primary                       |             | 0.624       | 0.373       | 0.373 |

Note:

TBN was measured pursuant to ASTM D2896, SASH was measured pursuant to ASTM D874, and soap content was measured pursuant to ASTM D3712

### Example 2

The Inventive and Comparative additive packages of Example 1 were formulated into passenger car motor oil lubricating compositions with API Group II and/or Group III base oils. The lubricants were then evaluated for average engine sludge merits pursuant to the Sequence VH test of ASTM D8256 and for average weighted piston deposits pursuant to the General Motors Oxidization and Deposit (GMOD) test of GMW-17043. The lubricants, base oil blends, and test results of the fluids are provided in Tables 4 (GMOD) and Table 5 (Sequence VH) below and FIGS. 1-3.

TABLE 4

| Weighted Piston Deposits (WPD) pursuant to GMW-17043. |           |          |           |      |
|-------------------------------------------------------|-----------|----------|-----------|------|
| Additive Package                                      | Viscosity | Group II | Group III | WPD  |
| Comparative                                           | 5W-30     | 36.9%    | 63.1%     | 3.78 |
| Inventive 2                                           | 5W-30     | 63.3%    | 36.7%     | 5.79 |
| Inventive 1                                           | 5W-30     | 60.9%    | 39.1%     | 5.41 |
| Comparative                                           | 5W-30     | —        | 100%      | 6.00 |

10

As shown in Table 4 and FIG. 1, when the comparative additive package was used in a 5W-30 lubricant having 100 percent of the API Group III oil, the 5W-30 lubricant had low levels of piston deposits as evidenced by a high WPD merit score (i.e., higher WPD merits reflects a cleaner piston with less deposits pursuant to GMW-17043). When the comparative additive package was used in a 5W-30 lubricant with a blend of API Group II and Group III base oils, the piston deposits increased as evidenced by a lower WPD merit score. However, when the Inventive additive packages were used with the blend of API Group II and Group III base oils, the piston cleanliness surprisingly increased with WPD merit scores comparable to the lubricant having 100% of the Group III base oil.

TABLE 5

| Average Engine Sludge (AES) pursuant to Sequence VH ASTM D8256 |           |          |           |      |
|----------------------------------------------------------------|-----------|----------|-----------|------|
| Additive Package                                               | Viscosity | Group II | Group III | AES  |
| Comparative                                                    | 0W-20     | —        | 100%      | 8.44 |
| Inventive 1                                                    | 0W-20     | 23.4%    | 76.6%     | 8.67 |
| Inventive 1                                                    | 5W-30     | 60.9%    | 39.1%     | 9.06 |
| Comparative                                                    | 5W-30     | —        | 100%      | 9.05 |
| Inventive 2                                                    | 5W-30     | 63.3%    | 36.7%     | 8.94 |
| Inventive 2                                                    | 5W-30     | 63.3%    | 36.7%     | 9.31 |
| Comparative                                                    | 5W-30     | —        | 100%      | 8.66 |
| Inventive 2                                                    | 0W-20     | 37.1%    | 62.9%     | 8.70 |
| Inventive 2                                                    | 0W-20     | 37.8%    | 62.2%     | 8.66 |
| Inventive 2                                                    | 0W-20     | 38.0     | 62.0      | 8.66 |
| Inventive 2                                                    | 0W-20     | 38.5     | 61.8      | 8.67 |

The results in Table 5 above and as shown in FIGS. 2 and 3 show that, when the Inventive additive packages were used in 5W-30 or 0W-20 lubricants including a blend of API Group II and Group III base oils, the inventive lubricants had average engine sludge (AES) ratings comparable to, and in some instances, surprisingly better than lubricants having only the higher quality Group III base oil.

It is noted that, as used in this specification and the appended claims, the singular forms "a," "an," and "the," include plural referents unless expressly and unequivocally limited to one referent. Thus, for example, reference to "an antioxidant" includes two or more different antioxidants. As used herein, the term "include" and its grammatical variants are intended to be non-limiting, such that recitation of items in a list is not to the exclusion of other like items that can be substituted or added to the listed items

For the purposes of this specification and appended claims, unless otherwise indicated, all numbers expressing quantities, percentages or proportions, and other numerical values used in the specification and claims, are to be understood as being modified in all instances by the term "about." Accordingly, unless indicated to the contrary, the numerical parameters set forth in the following specification and attached claims are approximations that can vary

depending upon the desired properties sought to be obtained by the present disclosure. At the very least, and not as an attempt to limit the application of the doctrine of equivalents to the scope of the claims, each numerical parameter should at least be construed in light of the number of reported significant digits and by applying ordinary rounding techniques.

It is to be understood that each component, compound, substituent or parameter disclosed herein is to be interpreted as being disclosed for use alone or in combination with one or more of each and every other component, compound, substituent or parameter disclosed herein.

It is further understood that each range disclosed herein is to be interpreted as a disclosure of each specific value within the disclosed range that has the same number of significant digits. Thus, for example, a range from 1 to 4 is to be interpreted as an express disclosure of the values 1, 2, 3 and 4 as well as any range of such values.

It is further understood that each lower limit of each range disclosed herein is to be interpreted as disclosed in combination with each upper limit of each range and each specific value within each range disclosed herein for the same component, compounds, substituent or parameter. Thus, this disclosure to be interpreted as a disclosure of all ranges derived by combining each lower limit of each range with each upper limit of each range or with each specific value within each range, or by combining each upper limit of each range with each specific value within each range. That is, it is also further understood that any range between the endpoint values within the broad range is also discussed herein. Thus, a range from 1 to 4 also means a range from 1 to 3, 1 to 2, 2 to 4, 2 to 3, and so forth.

Furthermore, specific amounts/values of a component, compound, substituent or parameter disclosed in the description or an example is to be interpreted as a disclosure of either a lower or an upper limit of a range and thus can be combined with any other lower or upper limit of a range or specific amount/value for the same component, compound, substituent or parameter disclosed elsewhere in the application to form a range for that component, compound, substituent or parameter.

While particular embodiments have been described, alternatives, modifications, variations, improvements, and substantial equivalents that are or can be presently unforeseen can arise to applicants or others skilled in the art. Accordingly, the appended claims as filed and as they can be amended are intended to embrace all such alternatives, modifications variations, improvements, and substantial equivalents.

What is claimed is:

1. A passenger car motor oil lubricating composition suitable for improving at least one of deposits, sludge, oxidization, and wear, the passenger car motor oil lubricating composition comprising:

a blend of base oils of lubricating viscosity including one or more API Group II base oils and one or more API Group III base oils and/or one or more API Group IV base oils;

oil soluble nitrogen-containing dispersant additives comprising (i) at least one boronated oil soluble nitrogen-containing dispersant additive and (ii) at least one non-boronated oil soluble nitrogen-containing dispersant additive wherein the oil soluble nitrogen-containing dispersant additives provide an amount of dispersant boron (B), an amount of dispersant nitrogen (N), and a dispersant total base number (TBN) to the passenger car motor oil lubricating composition,

wherein the dispersant TBN of the oil soluble nitrogen-containing dispersant additives is about 1.0 to about 1.28 mg KOH/gram as measured pursuant to ASTM D2896, and wherein the oil soluble nitrogen-containing dispersant additives provide no more than about 200 ppm of the dispersant boron to the passenger car motor oil lubricating composition;

metal-containing detergent additives including (i) at least one calcium-containing detergent additive and (ii) at least one magnesium-containing detergent additive; wherein the passenger car motor oil lubricating composition has a ratio of the dispersant boron, the dispersant nitrogen, and the dispersant TBN provided by the dispersant formula  $B/(N^*TBN)$  of less than 0.2.

2. The passenger car motor oil lubricating composition of claim 1, wherein the blend of base oils includes at least about 25 weight percent of the one or more API Group II base oils.

3. The passenger car motor oil lubricating composition of claim 1, wherein the blend of base oils includes at least about 50 weight percent of the one or more API Group II base oils.

4. The passenger car motor oil lubricating composition of claim 1, wherein the blend of base oils is about 25 to about 80 weight percent of the one or more API Group II base oils and about 20 to about 75 weight percent of the one or more API Group III base oils.

5. The passenger car motor oil lubricating composition of claim 1, wherein the nitrogen-containing dispersant additives provide up to 700 ppm dispersant nitrogen.

6. The passenger car motor oil lubricating composition of claim 1, wherein the nitrogen-containing dispersant additives provide up to 650 ppm dispersant nitrogen.

7. The passenger car motor oil lubricating composition of claim 1, wherein the metal-containing detergent additives provide an amount of calcium soap and an amount of magnesium soap to the passenger car motor oil lubricating composition and wherein the passenger car motor oil lubricating composition has more calcium soap than magnesium soap.

8. The passenger car motor oil lubricating composition of claim 7, wherein the metal-containing detergent additives have a weight ratio of the calcium soap to the magnesium soap of up to about 1.6:1.

9. The passenger car motor oil lubricating composition of claim 7, wherein the metal-containing detergent additives have a weight ratio of the calcium soap to the magnesium soap of up to about 1.4:1.

10. The passenger car motor oil lubricating composition of claim 7, wherein the metal-containing detergent additives are substantially free of detergent additives providing phenate soap.

11. The passenger car motor oil lubricating composition of claim 1, wherein the passenger car motor oil lubricating composition has an average engine sludge (AES) of at least about 7.6 merits as measured pursuant to ASTM D8256.

12. The passenger car motor oil lubricating composition of claim 1, wherein the passenger car motor oil lubricating composition has an average weighted piston deposits of at least 5.3 merits as measured pursuant to GMW-17043.

13. The passenger car motor oil lubricating composition of claim 1, further including a viscosity index improver having a shear stability index (SSI) of less than 50 as measured pursuant to ASTM D6278.

14. The passenger car motor oil lubricating composition of claim 13, wherein the viscosity index improver is a non-dispersant viscosity index improver selected from polyolefins, olefin copolymers, ethylene/propylene copolymers, polyisobutene, hydrogenated styrene-isoprene polymers,

styrene/maleic ester copolymers, hydrogenated styrene/butadiene copolymers, hydrogenated isoprene polymers, alpha-olefin maleic anhydride copolymers, polymethacrylates, polyacrylates, polyalkyl styrenes, hydrogenated alk-  
enyl aryl conjugated diene copolymers, and mixtures 5 thereof.

**15.** The passenger car motor oil lubricating composition of claim 1, wherein the lubricating composition has a sulfated ash (SASH) content of no more than about 0.9 weight percent as measured pursuant to ASTM D874. 10

**16.** The passenger car motor oil lubricating composition of claim 1, wherein the lubricating composition has a sulfated ash (SASH) content of no more than about 0.8 weight percent as measured pursuant to ASTM D874.

**17.** The passenger car motor oil lubricating composition 15 of claim 1, further including one or more metal dihydrocarbyl dithiophosphate compounds, wherein the hydrocarbyl groups thereof are derived from a mixture of secondary alcohols and primary alcohols and with a ratio of the primary alcohols to the secondary alcohols of about 0.3:1 to about 20 0.6:1.

**18.** The passenger car motor oil lubricating composition of claim 5, wherein an average number of carbon atoms in the hydrocarbyl groups per primary alcohol is no more than about 0.6:1. 25

\* \* \* \* \*